



US008382610B2

(12) **United States Patent**  
**Sullivan et al.**

(10) **Patent No.:** **US 8,382,610 B2**  
(45) **Date of Patent:** **Feb. 26, 2013**

- (54) **GOLF BALLS HAVING MULTI-LAYER CORES BASED ON POLYALKENAMER COMPOSITIONS**
- (75) Inventors: **Michael J. Sullivan**, Barrington, RI (US); **Brian Comeau**, Berkley, MA (US); **Douglas S. Goguen**, New Bedford, MA (US); **Robert Blink**, Newport, RI (US); **David A. Bulpett**, Boston, MA (US); **Mark L. Binette**, Mattapoisett, MA (US)
- (73) Assignee: **Acushnet Company**, Fairhaven, MA (US)
- (\*) Notice: Subject to any disclaimer, the term of this patent is extended or adjusted under 35 U.S.C. 154(b) by 288 days.

(21) Appl. No.: **12/870,926**(22) Filed: **Aug. 30, 2010**(65) **Prior Publication Data**

US 2010/0323820 A1 Dec. 23, 2010

**Related U.S. Application Data**

(63) Continuation-in-part of application No. 12/407,885, filed on Mar. 20, 2009, now Pat. No. 8,137,213, which is a continuation-in-part of application No. 11/972,240, filed on Jan. 10, 2008, now Pat. No. 7,722,482.

(51) **Int. Cl.**  
**A63B 37/06** (2006.01)

(52) **U.S. Cl.** ..... **473/376**(58) **Field of Classification Search** ..... **473/376, 473/373, 374**

See application file for complete search history.

(56) **References Cited**

## U.S. PATENT DOCUMENTS

- 2,998,977 A 9/1961 Molitor  
3,492,245 A 1/1970 Calderon  
3,804,803 A 4/1974 Streck

|              |         |                    |
|--------------|---------|--------------------|
| 4,183,876 A  | 1/1980  | Coran et al.       |
| 4,650,193 A  | 3/1987  | Molitor et al.     |
| 4,781,383 A  | 11/1988 | Kamada et al.      |
| 4,792,141 A  | 12/1988 | Llort              |
| 4,840,993 A  | 6/1989  | Bartz              |
| 4,858,924 A  | 8/1989  | Saito et al.       |
| 5,002,281 A  | 3/1991  | Nakahara et al.    |
| 5,033,748 A  | 7/1991  | Ebisuno            |
| 5,048,838 A  | 9/1991  | Chikaraishi et al. |
| 5,104,126 A  | 4/1992  | Gentiluomo         |
| 5,314,187 A  | 5/1994  | Proudfit           |
| 5,460,367 A  | 10/1995 | Horiuchi           |
| 5,482,285 A  | 1/1996  | Yabuki et al.      |
| 5,490,674 A  | 2/1996  | Hamada et al.      |
| 5,733,206 A  | 3/1998  | Nesbitt et al.     |
| 5,743,816 A  | 4/1998  | Ohsumi et al.      |
| 5,772,531 A  | 6/1998  | Ohsumi et al.      |
| 5,779,562 A  | 7/1998  | Melvin et al.      |
| 5,976,443 A  | 11/1999 | Nesbitt et al.     |
| 6,057,403 A  | 5/2000  | Sullivan et al.    |
| 6,071,201 A  | 6/2000  | Maruko             |
| 6,113,831 A  | 9/2000  | Nesbitt et al.     |
| 6,213,895 B1 | 4/2001  | Sullivan et al.    |
| 6,245,859 B1 | 6/2001  | Sullivan et al.    |
| 6,277,034 B1 | 8/2001  | Nesbitt et al.     |
| 6,336,872 B1 | 1/2002  | Moriyama et al.    |
| 6,379,269 B1 | 4/2002  | Nesbitt et al.     |
| 6,394,912 B1 | 5/2002  | Nakamura et al.    |

(Continued)

## OTHER PUBLICATIONS

EVONIK Industries, Product Information VESTENAMER 8012 Rubber with unique properties, Mar. 2009.

Primary Examiner — Raeann Gorden

(74) Attorney, Agent, or Firm — Daniel W. Sullivan

(57) **ABSTRACT**

The present invention generally relates to golf balls and more particularly to golf balls having multi-layered cores comprising a thermoset rubber center, a thermoplastic intermediate core layer, and a thermoset rubber outer core layer. A cover layer is disposed about the multi-layered core. At least one of the center, intermediate core layer, and outer core layer comprises a polyalkenamer rubber. The rubber composition helps improve resiliency of the core and provides the ball with a comfortable and soft feel.

**20 Claims, 1 Drawing Sheet**

## U.S. PATENT DOCUMENTS

|              |         |                 |                 |         |                 |
|--------------|---------|-----------------|-----------------|---------|-----------------|
| 6,406,383 B2 | 6/2002  | Moriyama et al. | 6,913,548 B2    | 7/2005  | Moriyama et al. |
| 6,431,998 B1 | 8/2002  | Nakamura et al. | 6,916,254 B2    | 7/2005  | Ladd et al.     |
| 6,432,342 B1 | 8/2002  | Nesbitt et al.  | 6,981,926 B2    | 1/2006  | Sullivan et al. |
| 6,500,076 B1 | 12/2002 | Morgan et al.   | 6,988,962 B2    | 1/2006  | Sullivan et al. |
| 6,569,036 B1 | 5/2003  | Takemura et al. | 7,037,965 B2    | 5/2006  | Sullivan et al. |
| 6,605,009 B1 | 8/2003  | Nakamura et al. | 7,041,009 B2    | 5/2006  | Sullivan et al. |
| 6,616,550 B2 | 9/2003  | Nesbitt et al.  | 7,044,864 B2    | 5/2006  | Sullivan et al. |
| 6,626,770 B2 | 9/2003  | Takemura et al. | 7,074,137 B2    | 7/2006  | Sullivan et al. |
| 6,767,940 B2 | 7/2004  | Voorheis et al. | 7,118,495 B2    | 10/2006 | Sullivan et al. |
| 6,783,468 B2 | 8/2004  | Sullivan et al. | 7,125,345 B2    | 10/2006 | Sullivan et al. |
| 6,815,521 B2 | 11/2004 | Iwami           | 7,153,467 B2    | 12/2006 | Brum et al.     |
| 6,852,044 B2 | 2/2005  | Sullivan et al. | 7,255,656 B2    | 8/2007  | Sullivan et al. |
| 6,855,074 B2 | 2/2005  | Kato            | 7,528,196 B2    | 5/2009  | Kim et al.      |
|              |         |                 | 2006/0128904 A1 | 6/2006  | Sullivan et al. |
|              |         |                 | 2009/0191981 A1 | 7/2009  | Kim et al.      |



## 1

**GOLF BALLS HAVING MULTI-LAYER  
CORES BASED ON POLYALKENAMER  
COMPOSITIONS**

**CROSS-REFERENCE TO RELATED  
APPLICATIONS**

This application is a continuation-in-part of co-assigned U.S. patent application Ser. No. 12/407,885 having a filing date of Mar. 20, 2009 now U.S. Pat. No. 8,137,213, which is a continuation-in-part of U.S. patent application Ser. No. 11/972,240, having a filing date of Jan. 10, 2008, now U.S. Pat. No. 7,722,482, the entire disclosures of which are hereby incorporated herein by reference.

**BACKGROUND OF THE INVENTION**

**1. Field of the Invention**

The present invention generally relates to golf balls, and more particularly to golf balls having multi-layer cores comprising a thermoset rubber center, a thermoplastic intermediate core layer, and a thermoset rubber outer core layer. In one preferred embodiment, at least one of the center, intermediate core layer, and outer core layer comprises a polyalkenamer rubber composition.

**2. Brief Review of the Related Art**

Golf balls having multi-layer cores are known. For example, U.S. Pat. No. 6,852,044 discloses golf balls having multi-layered cores having a relatively soft, low compression inner core surrounded by a relatively rigid outer core. U.S. Pat. No. 5,772,531 discloses a solid golf ball comprising a solid core having a three-layered structure composed of an inner layer, an intermediate layer, and an outer layer, and a cover for coating the solid core. U.S. Pat. No. 7,652,086 also discloses multi-layer core golf balls. Other examples of multi-layer cores can be found, for example, in U.S. Pat. Nos. 5,743,816, 6,071,201, 6,336,872, 6,379,269, 6,394,912, 6,406,383, 6,431,998, 6,569,036, 6,605,009, 6,626,770, 6,815,521, 6,855,074, 6,913,548, 6,981,926, 6,988,962, 7,074,137, 7,153,467 and 7,255,656.

Multi-piece golf balls having multi-layered cores and multi-layered covers may be made. The multi-layered cover includes inner and outer cover layers. The inner cover may be made of an olefin-based ionomer resin that imparts some hardness to the ball. These ionomer acid copolymers contain inter-chain ionic bonding and are generally made of an  $\alpha$ -olefin such as ethylene and a vinyl comonomer having an acid group such as methacrylic, acrylic acid, or maleic acid. Metal ions such as sodium, lithium, zinc, and magnesium are used to neutralize the acid groups in the copolymer. In recent years, there has been interest in using thermoplastic and thermosetting polyurethanes, polyureas, and hybrid compositions for the outer cover. The golf ball industry is looking to develop multi-piece balls having high resiliency as well as a soft feel. Balls having a high resiliency tend to reach a high velocity when struck by a golf club. As a result, the ball tends to travel a greater distance which is particularly important for driver shots off the tee. Meanwhile, the soft feel of the ball provides the player with a more enjoyable sensation when he/she strikes the ball with the club. The player senses a more natural feeling and control over the ball as the club face makes impact with the ball.

Kim et al., U.S. Pat. No. 7,528,196 and U.S. Patent Application Publication US 2009/0191981 disclose a golf ball comprising a core, cover layer, and optionally one or more inner cover layers, wherein at least one portion of the ball comprises a blend of a polyalkenamer and polyamide. The

## 2

polyalkenamer/polyamide composition contains about 2 to about 90 weight % of a polyalkenamer polymer and about 10 to about 98 weight % of a polyamide. The '196 patent and '981 Published Application further disclose that the polyalkenamer/polyamide composition may be blended with other polymers including polybutadiene, polyisoprene, polychloroprene, polybutylene, and styrene-butadiene rubber prior to molding. However, neither the '196 patent nor '981 Published Application discloses a multi-layered core having a thermoset rubber center, a thermoplastic intermediate core layer, and a thermoset rubber outer core layer, wherein at least one of the core layers is made of a polyalkenamer rubber composition.

In Voorheis et al., U.S. Pat. No. 6,767,940, a golf ball having a core, an intermediate layer, and a cover is disclosed. The core is formed from a composition containing an elastomeric polymer, free-radical initiator, and at least one stable free-radical. The stable free-radical increases the scorch time (time between start of reaction and onset of cross-linking) of the elastomeric polymer. The '940 patent discloses numerous materials that can be used to form the intermediate layer, which is distinguishable from the core, including natural rubbers; balata; gutta-percha; cis-polybutadienes; trans-polybutadienes; synthetic polyisoprenes; polyoctenamers; polypropylene resins; ionomer resins; polyamides; polyesters; urethanes; polyureas; chlorinated polyethylenes; polysulfide rubbers; and fluorocarbons.

In Sullivan et al., U.S. Pat. Nos. 6,783,468, 7041,009, 7,044,864, 7,118,495, and 7,125,345, a golf ball having a low compression and high coefficient of restitution (COR) layer supported and reinforced by a low deformation layer is disclosed. The preferred polymeric composition for the high COR layer is a base rubber compound, a co-reaction agent, a halogenated organosulfur compound, and a co-crosslinking or initiator agent. The low deformation layer may be made of rigid plastics or polymers reinforced with high strength organic or inorganic fillers or fibers. In one embodiment, the golf ball comprises an innermost core, an outer core, and a cover. The inner core comprises a low deformation material and the outer core comprises a rubber composition. The patents disclose that natural rubbers, including cis-polyisoprene, trans-polyisoprene or balata, synthetic rubbers including 1,2-polybutadiene, cis-polybutadiene, trans-polybutadiene, polychloroprene, poly(norbornene), polyoctenamer and polyoctenamer may be used for the outer core. However, there is no disclosure of forming a dual core, wherein the inner core has a positive hardness gradient and the outer core layer has a zero; negative; or positive hardness gradient, and the inner core and/or outer core is made of a polyalkenamer rubber composition.

In addition, Llort, U.S. Pat. No. 4,792,141 describes a balata-covered golf ball, where up to 40% of the balata used to form the cover has been replaced with polyoctenylene rubber. The golf ball contains a core and a cover wherein the cover is formed from a composition comprising about 97 to about 60 parts balata and about 3 to about 40 parts by weight polyoctenylene rubber based on 100 parts by weight polymer in the composition. The '141 patent discloses that using more than about 40 parts by weight of polyoctenylene produces deleterious effects.

The present invention provides a novel multi-layer core golf ball construction wherein the core comprises a thermoset rubber center, a thermoplastic intermediate core layer, and a thermoset rubber outer core layer. In a particularly preferred embodiment, at least one of the center, intermediate core layer, and outer core layer comprises a polyalkenamer rubber composition.

## SUMMARY OF THE INVENTION

In one embodiment, the present invention is directed to a golf ball comprising a center formed from a first thermoset rubber composition, an intermediate core layer formed from a thermoplastic composition, an outer core layer formed from a second thermoset rubber composition, and a cover layer. The center has a diameter of from 1.250 inches to 1.580 inches, a center hardness of from 40 Shore C to 70 Shore C, and a surface hardness of from 50 Shore C to 95 Shore C. The intermediate core layer has a thickness of 0.005 inches to 0.100 inches and a surface hardness of 60 Shore D or less. The outer core layer has a thickness of 0.010 inches to 0.100 inches and a surface hardness of 45 Shore C or greater. The cover layer has a thickness of from 0.010 inches to 0.050 inches and a surface hardness of 60 Shore D or greater. The specific gravity of at least one of the center, intermediate core layer, and outer core layer is less than 1.05 g/cc.

In another embodiment, the present invention is directed to a golf ball consisting essentially of a center formed from a first diene rubber composition, an intermediate core layer formed from a thermoplastic composition, an outer core layer formed from a second diene rubber composition, and a cover layer. The center has a diameter of from 1.350 inches to 1.490 inches, a center hardness of from 40 Shore C to 70 Shore C, and a surface hardness of from 70 Shore C to 90 Shore C. The intermediate core layer has a thickness of 0.005 inches to 0.100 inches and a surface hardness of 60 Shore D or less. The outer core layer has a thickness of 0.010 inches to 0.100 inches and a surface hardness of from 70 Shore C to 90 Shore C. The cover layer has a thickness of from 0.010 inches to 0.050 inches and a surface hardness of 60 Shore D or greater. The specific gravity of at least one of the center, intermediate core layer, and outer core layer is less than 1.05 g/cc.

In another embodiment, the present invention is directed to a golf ball comprising a center formed from a first thermoset rubber composition, an intermediate core layer formed from a thermoplastic composition, an outer core layer formed from a second thermoset rubber composition, and a cover layer. The center has a diameter of from 1.250 inches to 1.580 inches, a center hardness of from 40 Shore C to 70 Shore C, and a surface hardness of from 50 Shore C to 95 Shore C. The intermediate core layer has a thickness of 0.005 inches to 0.100 inches and a surface hardness of 60 Shore D or less. The outer core layer has a thickness of 0.010 inches to 0.100 inches and a surface hardness of 45 Shore C or greater. The cover layer has a thickness of from 0.010 inches to 0.050 inches and a surface hardness of 60 Shore D or greater. The specific gravity of at least one of the center, intermediate core layer, and outer core layer is greater than 1.25 g/cc.

In yet another embodiment, the present invention is directed to a golf ball consisting essentially of a center formed from a first diene rubber composition, an intermediate core layer formed from a thermoplastic composition, an outer core layer formed from a second diene rubber composition, and a cover layer. The center has a diameter of from 1.350 inches to 1.490 inches, a center hardness of from 40 Shore C to 70 Shore C, and a surface hardness of from 70 Shore C to 90 Shore C. The intermediate core layer has a thickness of 0.005 inches to 0.100 inches and a surface hardness of 60 Shore D or less. The outer core layer has a thickness of 0.010 inches to 0.100 inches and a surface hardness of from 70 Shore C to 90 Shore C. The cover layer has a thickness of from 0.010 inches to 0.050 inches and a surface hardness of 60 Shore D or greater. The specific gravity of at least one of the center, intermediate core layer, and outer core layer is greater than 1.25 g/cc.

In a particularly preferred embodiment, at least one of the center, intermediate core layer, and outer core layer comprises a polyalkenamer rubber composition as described in further detail below.

## BRIEF DESCRIPTION OF THE DRAWINGS

The novel features that are characteristic of the present invention are set forth in the appended claims. However, the preferred embodiments of the invention, together with further objects and attendant advantages, are best understood by reference to the following detailed description in connection with the accompanying drawings in which:

FIG. 1 is a cross-sectional view of a four-piece golf ball having a multi-layered core and a cover layer made in accordance with the present invention.

## DETAILED DESCRIPTION OF THE INVENTION

20 A golf ball having a multi-layer core and a cover enclosing the core is disclosed. The multi-layer core has an overall diameter. The multi-layer core comprises a center consisting of one or two thermoset rubber layers, a thermoplastic intermediate core layer, and a thermoset rubber outer core layer. 25 The multi-layer core has an overall diameter within a range having a lower limit of 1.000 or 1.300 or 1.400 or 1.500 or 1.600 or 1.610 inches and an upper limit of 1.620 or 1.630 or 1.640 inches. In a particular embodiment, the multi-layer core has an overall diameter of 1.500 inches or 1.510 inches or 30 1.530 inches or 1.550 inches or 1.570 inches or 1.580 inches or 1.590 inches or 1.600 inches or 1.610 inches or 1.620 inches.

The center may consist of one or two layers, each of which is formed from a thermoset rubber composition, and has an 35 overall diameter of 1.250 inches or greater, or 1.350 inches or greater, or 1.390 inches or greater, or 1.450 inches or greater, or an overall diameter within a range having a lower limit of 0.250 or 0.500 or 0.750 or 1.000 or 1.250 or 1.350 or 1.390 or 1.400 or 1.440 inches and an upper limit of 1.460 or 1.490 or 40 1.500 or 1.550 or 1.580 or 1.600 inches. In one embodiment, the center consists of a single layer formed from a thermoset rubber composition. In another embodiment, the center consists of two layers, each of which is formed from the same or 45 different thermoset rubber compositions. The center has a center hardness within a range having a lower limit of 20 or 25 or 30 or 35 or 40 or 45 or 50 or 55 Shore C and an upper limit of 60 or 65 or 70 or 75 or 90 Shore C. The center has an outer surface hardness within a range having a lower limit of 20 or 50 or 70 or 75 Shore C and an upper limit of 75 or 80 or 85 or 50 90 or 95 Shore C. The center has a negative hardness gradient, a zero hardness gradient, or a positive hardness gradient of up to 45 Shore C. The center has an overall compression of 90 or less, or 80 or less, or 70 or less, or 60 or less, or 50 or less, or 40 or less, or 20 or less, or a compression within a range 55 having a lower limit of 10 or 20 or 30 or 35 or 40 and an upper limit of 50 or 60 or 70 or 80 or 90.

Suitable rubber compositions for forming the center layer(s) comprise a base rubber, an initiator agent, a co-agent, and optionally one or more of a zinc oxide, zinc stearate or 60 stearic acid, antioxidant, and a soft and fast agent. Suitable base rubbers include natural and synthetic rubbers including, but not limited to, polybutadiene, polyisoprene, ethylene propylene rubber ("EPR"), styrene-butadiene rubber, styrenic block copolymer rubbers (such as SI, SIS, SB, SBS, SIBS, 65 and the like, where "S" is styrene, "I" is isobutylene, and "B" is butadiene), butyl rubber, halobutyl rubber, polystyrene elastomers, polyethylene elastomers, polyurethane elas-

tomers, polyurea elastomers, metallocene-catalyzed elastomers and plastomers, copolymers of isobutylene and para-alkylstyrene, halogenated copolymers of isobutylene and para-alkylstyrene, copolymers of butadiene with acrylonitrile, polychloroprene, alkyl acrylate rubber, chlorinated isoprene rubber, acrylonitrile chlorinated isoprene rubber, and combinations of two or more thereof. Diene rubbers are preferred, particularly polybutadiene, styrene-butadiene, and mixtures of polybutadiene with other elastomers wherein the amount of polybutadiene present is at least 40 wt % based on the total polymeric weight of the mixture. Particularly preferred polybutadienes include high-cis neodymium-catalyzed polybutadienes and cobalt-, nickel-, or lithium-catalyzed polybutadienes. Suitable examples of commercially available polybutadienes include, but are not limited to, Buna CB high-cis neodymium-catalyzed polybutadiene rubbers, such as Buna CB 23, and Taktene® high-cis cobalt-catalyzed polybutadiene rubbers, such as Taktene® 220 and 221, commercially available from LANXESS® Corporation; SE BR-1220, commercially available from The Dow Chemical Company; Europrene® NEOCIS® BR 40 and BR 60, commercially available from Polimeri Europa®; UBEPOL-BR® rubbers, commercially available from UBE Industries, Inc.; BR 01, commercially available from Japan Synthetic Rubber Co., Ltd.; and Neodene high-cis neodymium-catalyzed polybutadiene rubbers, such as Neodene BR 40, commercially available from Karbochem.

Suitable initiator agents include organic peroxides, high energy radiation sources capable of generating free radicals, and combinations thereof. High energy radiation sources capable of generating free radicals include, but are not limited to, electron beams, ultra-violet radiation, gamma radiation, X-ray radiation, infrared radiation, heat, and combinations thereof. Suitable organic peroxides include, but are not limited to, dicumyl peroxide; n-butyl-4,4-di(t-butylperoxy) valerate; 1,1-di(t-butylperoxy)3,3,5-trimethylcyclohexane; 2,5-dimethyl-2,5-di(t-butylperoxy) hexane; di-t-butyl peroxide; di-t-amyl peroxide; t-butyl peroxide; t-butyl cumyl peroxide; 2,5-dimethyl-2,5-di(t-butylperoxy)hexyne-3; di(2-t-butylperoxyisopropyl)benzene; dilauroyl peroxide; dibenzoyl peroxide; t-butyl hydroperoxide; lauryl peroxide; benzoyl peroxide; and combinations thereof. Examples of suitable commercially available peroxides include, but are not limited to Perkadox® BC dicumyl peroxide, commercially available from Akzo Nobel, and Varox® peroxides, such as Varox® ANS benzoyl peroxide and Varox® 231 1,1-di(t-butylperoxy)3,3,5-trimethylcyclohexane, commercially available from RT Vanderbilt Company, Inc. Peroxide initiator agents are generally present in the rubber composition in an amount of at least 0.05 parts by weight per 100 parts of the base rubber, or an amount within the range having a lower limit of 0.05 parts or 0.1 parts or 0.8 parts or 1 part or 1.25 parts or 1.5 parts by weight per 100 parts of the base rubber, and an upper limit of 2.5 parts or 3 parts or 5 parts or 6 parts or 10 parts or 15 parts by weight per 100 parts of the base rubber.

Co-agents are commonly used with peroxides to increase the state of cure. Suitable co-agents include, but are not limited to, metal salts of unsaturated carboxylic acids; unsaturated vinyl compounds and polyfunctional monomers (e.g., trimethylolpropane trimethacrylate); phenylene bismaleimide; and combinations thereof. Particular examples of suitable metal salts include, but are not limited to, one or more metal salts of acrylates, diacrylates, methacrylates, and dimethacrylates, wherein the metal is selected from magnesium, calcium, zinc, aluminum, lithium, nickel, and sodium. In a particular embodiment, the co-agent is selected from zinc salts of acrylates, diacrylates, methacrylates, dimethacry-

lates, and mixtures thereof. In another particular embodiment, the co-agent is zinc diacrylate. When the co-agent is zinc diacrylate and/or zinc dimethacrylate, the co-agent is typically included in the rubber composition in an amount within the range having a lower limit of 1 or 5 or 10 or 15 or 19 or 20 parts by weight per 100 parts of the base rubber, and an upper limit of 24 or 25 or 30 or 35 or 40 or 45 or 50 or 60 parts by weight per 100 parts of the base rubber. When one or more less active co-agents are used, such as zinc monomethacrylate and various liquid acrylates and methacrylates, the amount of less active co-agent used may be the same as or higher than for zinc diacrylate and zinc dimethacrylate co-agents. The desired compression may be obtained by adjusting the amount of crosslinking, which can be achieved, for example, by altering the type and amount of co-agent.

The rubber composition optionally includes a curing agent. Suitable curing agents include, but are not limited to, sulfur; N-oxydiethylene 2-benzothiazole sulfenamide; N,N-dio-ortho-tolylguanidine; bismuth dimethyldithiocarbamate; N-cyclohexyl 2-benzothiazole sulfenamide; N,N-diphenylguanidine; 4-morpholinyl-2-benzothiazole disulfide; dipentamethylenethiuram hexasulfide; thiuram disulfides; mercaptobenzothiazoles; sulfenamides; dithiocarbamates; thiuram sulfides; guanidines; thioureas; xanthates; dithiophosphates; aldehyde-amines; dibenzothiazyl disulfide; tetraethylthiuram disulfide; tetrabutylthiuram disulfide; and combinations thereof.

The rubber composition optionally contains one or more antioxidants. Antioxidants are compounds that can inhibit or prevent the oxidative degradation of the rubber. Some antioxidants also act as free radical scavengers; thus, when antioxidants are included in the rubber composition, the amount of initiator agent used may be as high or higher than the amounts disclosed herein. Suitable antioxidants include, for example, dihydroquinoline antioxidants, amine type antioxidants, and phenolic type oxidants.

The rubber composition may contain one or more fillers to adjust the density and/or specific gravity of the core. Exemplary fillers include precipitated hydrated silica, clay, talc, asbestos, glass fibers, aramid fibers, mica, calcium metasilicate, zinc sulfate, barium sulfate, zinc sulfide, lithopone, silicates, silicon carbide, diatomaceous earth, polyvinyl chloride, carbonates (e.g., calcium carbonate, zinc carbonate, barium carbonate, and magnesium carbonate), metals (e.g., titanium, tungsten, aluminum, bismuth, nickel, molybdenum, iron, lead, copper, boron, cobalt, beryllium, zinc, and tin), metal alloys (e.g., steel, brass, bronze, boron carbide whiskers, and tungsten carbide whiskers), oxides (e.g., zinc oxide, tin oxide, iron oxide, calcium oxide, aluminum oxide, titanium dioxide, magnesium oxide, and zirconium oxide), particulate carbonaceous materials (e.g., graphite, carbon black, cotton flock, natural bitumen, cellulose flock, and leather fiber), microballoons (e.g., glass and ceramic), fly ash, 55 regrind (i.e., core material that is ground and recycled), nanofillers and combinations thereof. The amount of particulate material(s) present in the rubber composition is typically within a range having a lower limit of 5 parts or 10 parts by weight per 100 parts of the base rubber, and an upper limit of 30 parts or 50 parts or 100 parts by weight per 100 parts of the base rubber. Filler materials may be dual-functional fillers, such as zinc oxide (which may be used as a filler/acid scavenger) and titanium dioxide (which may be used as a filler/brightener material).

The rubber composition may also contain one or more additives selected from processing aids, processing oils, plasticizers, coloring agents, fluorescent agents, chemical blow-

ing and foaming agents, defoaming agents, stabilizers, softening agents, impact modifiers, free radical scavengers, accelerators, scorch retarders, and the like. The amount of additive(s) typically present in the rubber composition is typically within a range having a lower limit of 0 parts by weight per 100 parts of the base rubber, and an upper limit of 20 parts or 50 parts or 100 parts or 150 parts by weight per 100 parts of the base rubber.

The rubber composition optionally includes a soft and fast agent. Preferably, the rubber composition contains from 0.05 phr to 10.0 phr of a soft and fast agent. In one embodiment, the soft and fast agent is present in an amount within a range having a lower limit of 0.05 or 0.1 or 0.2 or 0.5 phr and an upper limit of 1.0 or 2.0 or 3.0 or 5.0 phr. In another embodiment, the soft and fast agent is present in an amount of from 2.0 phr to 5.0 phr, or from 2.35 phr to 4.0 phr, or from 2.35 phr to 3.0 phr. In an alternative high concentration embodiment, the soft and fast agent is present in an amount of from 5.0 phr to 10.0 phr, or from 6.0 phr to 9.0 phr, or from 7.0 phr to 8.0 phr. In another embodiment, the soft and fast agent is present in an amount of 2.6 phr.

Suitable soft and fast agents include, but are not limited to, organosulfur and metal-containing organosulfur compounds; organic sulfur compounds, including mono, di, and polysulfides, thiol, and mercapto compounds; inorganic sulfide compounds; blends of an organosulfur compound and an inorganic sulfide compound; Group VIA compounds; substituted and unsubstituted aromatic organic compounds that do not contain sulfur or metal; aromatic organometallic compounds; hydroquinones; benzoquinones; quinhydrone; catechols; resorcinols; and combinations thereof.

Preferably, the halogenated thiophenol compound is pentachlorothiophenol, which is commercially available in neat form or under the tradename STRUKTOL®, a clay-based carrier containing the sulfur compound pentachlorothiophenol loaded at 45 percent (correlating to 2.4 parts PCTP). STRUKTOL® is commercially available from Struktol Company of America of Stow, Ohio. PCTP is commercially available in neat form from eChinachem of San Francisco, Calif. and in the salt form from eChinachem of San Francisco, Calif. Most preferably, the halogenated thiophenol compound is the zinc salt of pentachlorothiophenol, which is commercially available from eChinachem of San Francisco, Calif. Suitable organosulfur compounds are further disclosed, for example, in U.S. Pat. Nos. 6,635,716, 6,919,393, 7,005,479 and 7,148, 279, the entire disclosures of which are hereby incorporated herein by reference. In a particular embodiment, the soft and fast agent is selected from ZnPCTP, PCTP, ditolyl disulfide, diphenyl disulfide, dixylyl disulfide, 2-nitroresorcinol, and combinations thereof.

Suitable types and amounts of base rubber, initiator agent, co-agent, filler, and additives are more fully described in, for example, U.S. Pat. Nos. 6,566,483, 6,695,718, 6,939,907, 7,041,721 and 7,138,460, the entire disclosures of which are hereby incorporated herein by reference. Particularly suitable diene rubber compositions are further disclosed, for example, in U.S. Pat. No. 7,654,918, the entire disclosure of which is hereby incorporated herein by reference.

The intermediate core layer is formed from a thermoplastic composition and has a thickness within a range having a lower limit of 0.005 or 0.010 or 0.020 or 0.040 inches and an upper limit of 0.050 or 0.060 or 0.070 or 0.080 or 0.090 or 0.100 inches. In one embodiment, the intermediate core layer has a surface hardness of 25 Shore C or greater, or 40 Shore C or greater, or a surface hardness within a range having a lower limit of 25 or 30 or 35 Shore C and an upper limit of 80 or 85 Shore C. In another embodiment, the intermediate core layer

has a surface hardness of 60 Shore D or less, or a surface hardness within a range having a lower limit of 20 or 30 or 35 or 45 Shore D and an upper limit of 55 or 60 or 65 Shore D. In yet another embodiment, the surface hardness of the intermediate layer is greater than the surface hardness of both the center and the outer core layer.

Suitable thermoplastic compositions for forming the intermediate core layer include, but are not limited to, partially- and fully-neutralized ionomers, graft copolymers of ionomer and polyamide, and the following non-ionomeric polymers, including homopolymers and copolymers thereof, as well as their derivatives that are compatibilized with at least one grafted or copolymerized functional group, such as maleic anhydride, amine, epoxy, isocyanate, hydroxyl, sulfonate, phosphonate, and the like:

- (a) polyesters, particularly those modified with a compatibilizing group such as sulfonate or phosphonate, including modified poly(ethylene terephthalate), modified poly(butylene terephthalate), modified poly(propylene terephthalate), modified poly(trimethylene terephthalate), modified poly(ethylene naphthalene), and those disclosed in U.S. Pat. Nos. 6,353,050, 6,274,298, and 6,001,930, the entire disclosures of which are hereby incorporated herein by reference, and blends of two or more thereof;
- (b) polyamides, polyamide-ethers, and polyamide-esters, and those disclosed in U.S. Pat. Nos. 6,187,864, 6,001, 930, and 5,981,654, the entire disclosures of which are hereby incorporated herein by reference, and blends of two or more thereof;
- (c) polyurethanes, polyureas, polyurethane-polyurea hybrids, and blends of two or more thereof;
- (d) fluoropolymers, such as those disclosed in U.S. Pat. Nos. 5,691,066, 6,747,110 and 7,009,002, the entire disclosures of which are hereby incorporated herein by reference, and blends of two or more thereof;
- (e) non-ionomeric acid polymers, such as E/Y- and E/X/Y-type copolymers, wherein E is an olefin (e.g., ethylene), Y is a carboxylic acid such as acrylic, methacrylic, crotonic, maleic, fumaric, or itaconic acid, and X is a softening comonomer such as vinyl esters of aliphatic carboxylic acids wherein the acid has from 2 to 10 carbons, alkyl ethers wherein the alkyl group has from 1 to 10 carbons, and alkyl alkylacrylates such as alkyl methacrylates wherein the alkyl group has from 1 to 10 carbons; and blends of two or more thereof;
- (f) metallocene-catalyzed polymers, such as those disclosed in U.S. Pat. Nos. 6,274,669, 5,919,862, 5,981, 654, and 5,703,166, the entire disclosures of which are hereby incorporated herein by reference, and blends of two or more thereof;
- (g) polystyrenes, such as poly(styrene-co-maleic anhydride), acrylonitrile-butadiene-styrene, poly(styrene sulfonate), polyethylene styrene, and blends of two or more thereof;
- (h) polypropylenes and polyethylenes, particularly grafted polypropylene and grafted polyethylenes that are modified with a functional group, such as maleic anhydride of sulfonate, and blends of two or more thereof;
- (i) polyvinyl chlorides and grafted polyvinyl chlorides, and blends of two or more thereof;
- (j) polyvinyl acetates, preferably having less than about 9% of vinyl acetate by weight, and blends of two or more thereof;

- (k) polycarbonates, blends of polycarbonate/acrylonitrile-butadiene-styrene, blends of polycarbonate/polyurethane, blends of polycarbonate/polyester, and blends of two or more thereof;
- (l) polyvinyl alcohols, and blends of two or more thereof;
- (m) polyethers, such as polyarylene ethers, polyphenylene oxides, block copolymers of alkenyl aromatics with vinyl aromatics and poly(amic ester)s, and blends of two or more thereof;
- (n) polyimides, polyetherketones, polyamideimides, and blends of two or more thereof;
- (o) polycarbonate/polyester copolymers and blends; and
- (p) combinations of any two or more of the above thermoplastic polymers.

Ionomeric compositions suitable for forming the intermediate core layer comprise one or more acid polymers, each of which is partially- or fully-neutralized, and optionally additives, fillers, and/or melt flow modifiers. Suitable acid polymers are salts of homopolymers and copolymers of  $\alpha,\beta$ -ethylenically unsaturated mono- or dicarboxylic acids, and combinations thereof, optionally including a softening monomer, and preferably having an acid content (prior to neutralization) of from 1 wt % to 30 wt %, more preferably from 5 wt % to 20 wt %. The acid polymer is preferably neutralized to 70% or higher, including up to 100%, with a suitable cation source, such as metal cations and salts thereof, organic amine compounds, ammonium, and combinations thereof. Preferred cation sources are metal cations and salts thereof, wherein the metal is preferably lithium, sodium, potassium, magnesium, calcium, barium, lead, tin, zinc, aluminum, manganese, nickel, chromium, copper, or a combination thereof. Suitable additives and fillers include, for example, blowing and foaming agents, optical brighteners, coloring agents, fluorescent agents, whitening agents, UV absorbers, light stabilizers, defoaming agents, processing aids, mica, talc, nanofillers, antioxidants, stabilizers, softening agents, fragrance components, plasticizers, impact modifiers, acid copolymer wax, surfactants; inorganic fillers, such as zinc oxide, titanium dioxide, tin oxide, calcium oxide, magnesium oxide, barium sulfate, zinc sulfate, calcium carbonate, zinc carbonate, barium carbonate, mica, talc, clay, silica, lead silicate, and the like; high specific gravity metal powder fillers, such as tungsten powder, molybdenum powder, and the like; regrind, i.e., core material that is ground and recycled; and nano-filters.

Suitable melt flow modifiers include, for example, fatty acids and salts thereof, polyamides, polyesters, polyacrylates, polyurethanes, polyethers, polyureas, polyhydric alcohols, and combinations thereof. Suitable ionomeric compositions include blends of highly neutralized polymers (i.e., neutralized to 70% or higher) with partially neutralized ionomers as disclosed, for example, in U.S. Pat. No. 7,652,086, the entire disclosure of which is hereby incorporated herein by reference. Suitable ionomeric compositions also include blends of one or more partially- or fully-neutralized polymers with additional thermoplastic and thermoset materials, including, but not limited to, non-ionomeric acid copolymers, engineering thermoplastics, fatty acid/salt-based highly neutralized polymers, polybutadienes, polyurethanes, polyureas, polyesters, polycarbonate/polyester blends, thermoplastic elastomers, maleic anhydride-grafted metallocene-catalyzed polymers, and other conventional polymeric materials. Suitable ionomeric compositions are further disclosed, for example, in U.S. Pat. Nos. 6,653,382, 6,756,436, 6,777,472, 6,894,098, 6,919,393, and 6,953,820, the entire disclosures of which are hereby incorporated herein by reference.

- Examples of commercially available thermoplastics suitable for forming the intermediate core layer include, but are not limited to, Pebax® thermoplastic polyether block amides, commercially available from Arkema Inc.; Surlyn® ionomer resins, Hytrel® thermoplastic polyester elastomers, and ionomeric materials sold under the trade names DuPont® HPF 1000 and HPF 2000, all of which are commercially available from E. I. du Pont de Nemours and Company; Iotek® ionomers, commercially available from ExxonMobil Chemical Company; Amplify® IO ionomers of ethylene acrylic acid copolymers, commercially available from The Dow Chemical Company; Clarix® ionomer resins, commercially available from A. Schulman Inc.; Elastollan® polyurethane-based thermoplastic elastomers, commercially available from BASF; and Xylex® polycarbonate/polyester blends, commercially available from SABIC Innovative Plastics.

Also suitable for forming the intermediate core layer are the thermoplastic compositions disclosed herein as suitable for forming cover layers. In a particular embodiment, the intermediate core layer is formed from a blend of two or more ionomers. In a particular aspect of this embodiment, the intermediate core layer is fainted from a 50 wt %/50 wt % blend of two different partially-neutralized ethylene/methacrylic acid copolymers.

In another particular embodiment, the intermediate core layer is formed from a blend of one or more ionomers and a maleic anhydride-grafted non-ionomeric polymer. In a particular aspect of this embodiment, the non-ionomeric polymer is a metallocene-catalyzed polymer. In another particular aspect of this embodiment, the intermediate core layer is formed from a blend of a partially-neutralized ethylene/methacrylic acid copolymer and a maleic anhydride-grafted metallocene-catalyzed polyethylene.

In yet another particular embodiment, the intermediate core layer is formed from a composition selected from the group consisting of partially- and fully-neutralized ionomers optionally blended with a maleic anhydride-grafted non-ionomeric polymer; polyester elastomers; polyamide elastomers; and combinations of two or more thereof.

The thermoplastic intermediate core layer is optionally treated or admixed with a thermoset diene composition to reduce or prevent flow upon overmolding. Optional treatments may also include the addition of peroxide to the material prior to molding, or a post-molding treatment with, for example, a crosslinking solution, electron beam, gamma radiation, isocyanate or amine solution treatment, or the like. Such treatments may prevent the intermediate layer from melting and flowing or "leaking" out at the mold equator, as the thermoset outer core layer is molded thereon at a temperature necessary to crosslink the outer core layer, which is typically from 280° F. to 360° F. for a period of about 5 to 30 minutes. Suitable thermoplastic intermediate core layer compositions are further disclosed, for example, in U.S. Pat. Nos. 5,919,100, 6,872,774 and 7,074,137, the entire disclosures of which are hereby incorporated herein by reference.

The outer core layer is formed from a thermoset rubber composition and has a thickness within a range having a lower limit of 0.010 or 0.020 or 0.025 or 0.030 or 0.035 inches and an upper limit of 0.040 or 0.070 or 0.075 or 0.080 or 0.100 or 0.150 inches. In a particular embodiment, the outer core layer has a thickness of 0.035 inches or 0.040 inches or 0.045 inches or 0.050 inches or 0.055 inches or 0.060 inches or 0.065 inches.

In one embodiment, the outer core layer has a surface hardness of 45 Shore C or greater, or 70 Shore C or greater, or 75 Shore C or greater, or 80 Shore C or greater, or a surface hardness within a range having a lower limit of 45 or 70 or 80

## 11

Shore C and an upper limit of 90 or 95 Shore C. In a particular aspect of this embodiment, the surface hardness of the outer core layer is greater than the surface hardness of the center. In another particular aspect of this embodiment, the surface hardness of the outer core layer is less than the surface hardness of the center.

In another embodiment, the outer core layer has a surface hardness of 20 Shore C or greater, or 30 Shore C or greater, or 35 Shore C or greater, or 40 Shore C or greater, or a surface hardness within a range having a lower limit of 20 or 30 or 35 or 40 or 50 Shore C and an upper limit of 60 or 70 or 80 Shore C. In a particular aspect of this embodiment, the outer core layer is formed from a rubber composition selected from those disclosed in U.S. Pat. Nos. 7,537,530 and 7,537,529, the entire disclosures of which are hereby incorporated herein by reference.

Suitable rubber compositions for forming the outer core layer include the rubber compositions disclosed above for forming the center layer(s). The outer core layer composition may be the same or a different rubber composition than the composition(s) used to form the center layer(s). Either of the center layer(s) or outer core layer may further comprise from 1 to 100 phr of a stiffening agent. Preferably, if present, the stiffening agent is present in the outer core layer composition and not the inner core layer composition. Suitable stiffening agents include, but are not limited to, ionomers, acid copolymers and terpolymers, polyamides, and polyesters. Stiffening agents are further disclosed, for example, in U.S. Pat. Nos. 6,120,390 and 6,284,840, the entire disclosures of which are hereby incorporated herein by reference. A transpolyisoprene (e.g., TP-301 transpolyisoprene, commercially available from Kuraray Co., Ltd.) or transbutadiene rubber may also be added to increase stiffness to a core layer and/or improve cold-forming properties, which may improve processability by making it easier to mold outer core layer half-shells during the golf ball manufacturing process. When included in a core layer composition, the stiffening agent is preferably present in an amount of from 5 to 10 pph.

In one embodiment, the specific gravity of one or more of the core layers is increased. Suitable fillers for increasing specific gravity include, but are not limited to, metal and metal alloy powders, including, but not limited to, bismuth powder, boron powder, brass powder, bronze powder, cobalt powder, copper powder, nickel-chromium iron metal powder, iron metal powder, molybdenum powder, nickel powder, stainless steel powder, titanium metal powder zirconium oxide powder, tungsten metal powder, beryllium metal powder, zinc metal powder, and tin metal powder; metal flakes, including, but not limited to, aluminum flakes; metal oxides, including, but not limited to, zinc oxide, iron oxide, aluminum oxide, titanium dioxide, magnesium oxide, zirconium oxide, and tungsten trioxide; metal stearates; particulate carbonaceous materials, including, but not limited to, graphite and carbon black; and nanoparticulates and hybrid organic/inorganic materials, such as those disclosed in U.S. Pat. Nos. 6,793,592 and 6,919,395, the entire disclosures of which are hereby incorporated herein by reference. Particularly suitable density-increasing fillers include, but are not limited to, tungsten, tungsten oxide, tungsten metal powder, zinc oxide, barium sulfate, and titanium dioxide.

In another embodiment, the specific gravity of one or more of the core layers is reduced. The specific gravity of a layer can be reduced by incorporating cellular resins, low specific gravity fillers, fibers, flakes, or spheres, or hollow microspheres or balloons, such as glass bubbles or ceramic zeo-spheres, in the polymeric matrix. The specific gravity of a layer can also be reduced by foaming. Typical physical foam-

## 12

ing/blowing agents include volatile liquids such as freons (CFCs), other halogenated hydrocarbons, water, aliphatic hydrocarbons, gases, and solid blowing agents, i.e., compounds that liberate gas as a result of desorption of gas. 5 Typical chemical foaming/blowing agents include inorganic agents, such as ammonium carbonate and carbonates of alkali metals, and organic agents, such as azo and diazo compounds. Suitable azo compounds include, but are not limited to, 2,2'-azobis(2-cyanobutane), 2,2'-azobis(methylbutyronitrile), 10 azodicarbonamide, p,p'-oxybis(benzene sulfonyl hydrazide), p-toluene sulfonyl semicarbazide, and p-toluene sulfonyl hydrazide. Blowing agents also include Celogen® foaming/blowing agents, commercially available from Lion Copolymer, LLC; Opex® foaming/blowing agents, commercially 15 available from Chemtura Corporation; nitroso compounds, sulfonylhydrazides, azides of organic acids and their analogs, triazines, tri- and tetrazole derivatives, sulfonyl semicarbazides, urea derivatives, guanidine derivatives, and esters such as alkoxyboroxines. Blowing agents also include agents that 20 liberate gasses as a result of chemical interaction between components, such as mixtures of acids and metals, mixtures of organic acids and inorganic carbonates, mixture of nitriles and ammonium salts, and the hydrolytic decomposition of urea. Suitable foaming/blowing agents also include expandable microspheres, such as EXPANCEL® microspheres, 25 commercially available from Akzo Nobel.

In yet another embodiment, the specific gravity of one or more of the core layers is increased and the specific gravity of one or more of the core layers is reduced. Methods and 30 materials for adjusting the specific gravity of a golf ball layer are further disclosed, for example, in U.S. Pat. Nos. 6,494,795; 6,688,991; 6,692,380; 6,995,191; 7,259,191; 7,452,291; 7,651,415; and 7,708,654, the entire disclosures of which are hereby incorporated herein by reference.

The specific gravity of each of the core layers is from 0.50 g/cc to 5.00 g/cc. Core layers having an increased specific gravity preferably have a specific gravity of 1.15 g/cc or greater, or 1.20 g/cc or greater, or 1.25 g/cc or greater, or 1.30 g/cc or greater, or 1.35 g/cc or greater, or 1.40 g/cc or greater, 40 or 1.50 g/cc or greater. Core layers having a reduced specific gravity preferably have a specific gravity of 1.05 g/cc or less, or 0.95 g/cc or less, or 0.90 g/cc or less, or 0.85 g/cc or less.

In a particular embodiment, the specific gravity of the center is 0.95 g/cc or less or 0.90 g/cc or less; the specific 45 gravity of the intermediate layer is 1.00 g/cc or less, or 0.95 g/cc or less, or from 0.90 g/cc to 1.00 g/cc; and the specific gravity of the outer core layer is 1.25 g/cc or greater, or greater than 1.25 g/cc, or 1.30 g/cc or greater. In a particular aspect of this embodiment, the specific gravity of the center is less than the specific gravity of the intermediate layer. In another particular aspect of this embodiment, the center is formed from a composition wherein the specific gravity has been reduced, the intermediate core layer is formed from a composition wherein the specific gravity has not been modified, and the outer core layer is formed from a composition wherein the specific gravity has been increased.

In one preferred embodiment, a rubber composition comprising "cycloalkene rubber" may be used to make at least one section (center, intermediate, or outer layer) of the core. In 60 accordance with the present invention, it now has been found that rubber compositions comprising "cycloalkene rubber" can be used to provide a golf ball having improved resiliency and rebounding properties along with a soft feel. Cycloalkene rubbers are rubbery polymers made from one or more cycloalkenes having from 5 to 20, preferably 5 to 15, ring carbon atoms. The cycloalkene rubbers (also referred to as polyalkenylene or polyalkenamer rubbers) may be prepared

by ring opening metathesis polymerization of one or more cycloalkenes in the presence of organometallic catalysts as is known in the art. Such polymerization methods are disclosed, for example, in U.S. Pat. Nos. 3,492,245 and 3,804,803, the disclosures of which are hereby incorporated by reference. By the term, "cycloalkene rubber" as used herein, it is meant a compound having at least 20 weight % macrocycles (cyclic content). The cyclic and linear portions of the cycloalkene rubber have the following general chemical structures:



Suitable cyclic olefins that can be used to make the cycloalkene rubber include unsaturated hydrocarbons with 4 to 12 ring carbon atoms in one or more rings e.g., 1-3 rings, which exhibit in at least one ring an unsubstituted double bond which is not in conjugation to a second double bond which may be present and which may have any degree of substitution; the substituents must not interfere with the metathesis catalysts and are preferably alkyl groups of 1 to 4 carbon atoms or a part of a cyclic structure of 4 to 8 carbon atoms. Examples are cyclobutene, cyclopentene, cycloheptene, cis- and trans-cyclooctene, cyclononene, cyclodecene, cycloundecene, cis- and trans-cyclododecene, cis, cis-cyclooctadiene, 1-methyl-1,5-cyclooctadiene, 3-methyl-1,5-cyclooctadiene, and 3,7-dimethyl-1,5-cyclooctadiene.

Examples of suitable polyalkenamer rubbers are polypentenamer rubber, polyheptenamer rubber, polyoctenamer rubber, polydecenamer rubber and polydodecenamer rubber. Polyoctenamer rubbers are commercially available from Evonik Degussa GmbH of Marl, Germany and sold under the VESTENAMER tradename. The polyalkenamer rubber used in the present invention preferably has a trans-bond content of about 55% or greater and a second heat melting point of about 30° C. or greater. More preferably, the cycloalkene rubber has a trans-bond content of 75% or greater and a second heat melting point of 50° C. or greater. Furthermore, the polyalkenamer rubber material preferably has a molecular weight of about 80,000 or greater (measured according to GPC); a glass transition temperature (Tg) of about 55° C. or less (measured according to ISO 6721 or 4663); a cis-to-trans ratio of double bonds of about 40:60 or preferably about 20:80 (measured according to IR); a Mooney viscosity ML (1+4) 100° C. of less than about 10 (measured according to DIN 53 523 or ASTM-D 1646); a viscosity number J/23° C. of about 130 or preferably about 120 ml/g (measured according to ISO 1628-

1); and a density of about 0.9 g/cm<sup>3</sup> or greater (measured according to DIN 53 479 A or ISO 1183).

The polyalkenamer rubber compound, of and by itself, has relatively high crystallinity. For example, a specific grade of polyalkenamer rubber (VESTENAMER 8012) has a crystallinity of approximately 30% (measured by DSC, second melting.) The ratio of cis double bonds to trans double bonds (cis/trans ratio) in the polymer is significant in determining the degree of crystallinity in the polymer. In general, if the trans-bond content of the polymer is relatively high, the crystallinity and melting point of the polymer is relatively high. That is, as the trans-bond content increases, the crystallinity of the polymer increases. The polyalkenamer rubber, VESTENAMER 8012 has a trans-bond content of about 80%. In accordance with the present invention, it has been found the compression of polyalkenamer rubber cores is reduced and the Coefficient of Restitution ("COR") of the cores is increased when the rubber composition is cross-linked to a relatively high degree and the composition does not contain a reactive cross-linking co-agent such as zinc diacrylate (ZDA). The polyalkenamer rubber composition may be cured using a conventional curing process such as peroxide-curing, sulfur-curing, and high-energy radiation, and combinations thereof. For example, the composition may be peroxide-cured. When peroxide is added at relatively high amounts (particularly, at least 2.5 and preferably 5.0 phr) and the composition (which if it does not contain a reactive cross-linking co-agent such as ZDA) is cured to cross-link the rubber chains, then the compression of the polyalkenamer rubber cores is reduced and the COR of the cores is increased. It is believed this phenomenon is due, at least in part, to disrupting the crystalline structure of the polymer by curing and cross-linking the composition in accordance with this invention. While not wishing to be bound by any theory, it is believed the cross-linking causes the tightly packed structures within the mass of polyalkenamer polymer to spread out, thus disrupting the crystallinity of the material. It appears the crystallinity may be partially disrupted and the polymer remains in a partially crystalline state. As a result, the polyalkenamer rubber (which if it does not contain a reactive cross-linking agent such as ZDA) becomes softer and more rubbery and the compression of core samples made from the composition decreases.

One example of a commercially-available material that can be used in accordance with this invention is VESTENAMER 8012 (trans-bond content of about 80% and a melting point of about 54° C.). The material, VESTENAMER 6213 (trans-bond content of about 60% and a melting point of about 30° C.) also may be effective.

In the present invention, it has been found that rubber compositions comprising polyoctenamer rubber are particularly effective. Polyoctenamer rubber compositions can be used to make a core that provides the golf ball with good rebounding properties (distance) without sacrificing a nice feel to the ball. The resulting ball has a relatively high COR allowing it to reach a high velocity when struck by a golf club. Thus, the ball tends to travel a greater distance which is particularly important for driver shots off the tee. Meanwhile, the soft feel of the ball provides the player with a more pleasant sensation when he/she strikes the ball with the club. The player senses more control over the ball as the club face makes impact. Furthermore, the soft feel of the ball's cover allows players to place a spin on the ball and better control its flight pattern which is particularly important for approach shots near the green.

The polyalkenamer rubber is used in an amount of at least 50% by weight based on total amount of polymer in the

## 15

rubber composition used to make the core. Preferably, the polyalkenamer rubber is present in an amount of 65 to 100% by weight and more preferably 75 to 100% by weight based on total polymer weight. It is believed that when the concentration of the polyalkenamer rubber is less than 50% by weight, the resiliency of the rubber composition is not significantly improved. In particular versions, the blend may contain a lower concentration of polyalkenamer rubber in the amount of 50%, 55%, 60%, 65%, or 70% and an upper concentration of polyalkenamer in the amount of 75%, 80%, 85%, 90%, or 95%.

The polyalkenamer rubber may be blended with other rubber and polymeric materials. As described above, these rubber materials include, but are not limited to, polybutadiene, polyisoprene, ethylene propylene rubber ("EPR"), ethylene propylene diene rubber ("EPDM"), styrene-butadiene rubber, styrenic block copolymer rubbers (such as SI, SIS, SB, SBS, SIBS, SEBS, and the like, where "S" is styrene, "I" is isobutylene, "B" is butadiene, and "E" is ethylene), butyl rubber, halobutyl rubber, polystyrene elastomers, polyethylene elastomers, polyurethane elastomers, polyurea elastomers, metallocene-catalyzed elastomers and plastomers, copolymers of isobutylene and para-alkylstyrene, halogenated copolymers of isobutylene and para-alkylstyrene, copolymers of butadiene with acrylonitrile, polychloroprene, alkyl acrylate rubber, chlorinated isoprene rubber, acrylonitrile chlorinated isoprene rubber, and combinations of two or more thereof. A preferred base rubber is 1,4-polybutadiene having a cis-bond structure of at least 40%, preferably greater than 80%, and more preferably greater than 90%.

Examples of commercially available polybutadiene rubbers that can be used in accordance with this invention include, but are not limited to, BUNA® CB22 and BUNA® CB23, commercially available from Lanxess Corp.; UBE-POL® 360L and UBEPOL® 150L and UBEPOL-BR rubbers, commercially available from UBE Industries, Ltd. of Tokyo, Japan; KINEX® 7245 and KINEX® 7265, commercially available from Goodyear of Akron, Ohio; SE BR-1220, and BUNA® CB1203G1, CB1220, and CB1221, commercially available from Lanxess Corp.; EUROPRENE® NEO-CIS® BR 40 and BR 60, commercially available from Polimeri Europa; and BR 01, BR 730, BR 735, BR 11, and BR 51, commercially available from Japan Synthetic Rubber Co., Ltd; and Afdene 45, Afdene 50, Neodene 40, and Neodene 45, commercially available from Karbochem (PTY) Ltd. of Bruma, South Africa.

As discussed above, the polyalkenamer rubber composition may be cured using a conventional curing process. Suitable curing processes include, for example, peroxide-curing, sulfur-curing, high-energy radiation, and combinations thereof. Preferably, the rubber composition contains a free-radical initiator selected from organic peroxides, high energy radiation sources capable of generating free-radicals, and combinations thereof. In one preferred version, the rubber composition is peroxide-cured. Suitable organic peroxides include, but are not limited to, dicumyl peroxide; n-butyl-4, 4-di(t-butylperoxy) valerate; 1,1-di(t-butylperoxy)3,3,5-trimethylcyclohexane; 2,5-dimethyl-2,5-di(t-butylperoxy)hexane; di-t-butyl peroxide; di-t-amyl peroxide; t-butyl peroxide; t-butyl cumyl peroxide; 2,5-dimethyl-2,5-di(t-butylperoxy)hexyne-3; di(2-t-butyl-peroxyisopropyl)benzene; dilauroyl peroxide; dibenzoyl peroxide; t-butyl hydroperoxide; and combinations thereof. In a particular embodiment, the free radical initiator is dicumyl peroxide, including, but not limited to Perkadox® BC, commercially available from Akzo Nobel. Peroxide free-radical initiators are generally present in the rubber composition in an amount of at least 0.05

## 16

parts by weight per 100 parts of the base rubber, or an amount within the range having a lower limit of 0.05 parts or 0.1 parts or 1 part or 1.25 parts or 1.5 parts or 2.5 parts or 5 parts by weight per 100 parts of the total rubbers, and an upper limit of 2.5 parts or 3 parts or 5 parts or 6 parts or 10 parts or 15 parts by weight per 100 parts of the base rubber. In one preferred version, the peroxide free-radical initiator is present in an amount of at least 2.5 and more preferably 5 parts per hundred (phr). As further discussed in the Examples below, it is believed the high crystallinity of the polyalkenamer rubber is reduced by adding the peroxide at relatively high amounts to the rubber composition and curing the composition so it is cross-linked.

The polyalkenamer rubber composition may further include a reactive cross-linking co-agent. Suitable co-agents include, but are not limited to, metal salts of unsaturated carboxylic acids having from 3 to 8 carbon atoms; unsaturated vinyl compounds and polyfunctional monomers (e.g., trimethylolpropane trimethacrylate); phenylene bismaleimide; and combinations thereof. Particular examples of suitable metal salts include, but are not limited to, one or more metal salts of acrylates, diacrylates, methacrylates, and dimethacrylates, wherein the metal is selected from magnesium, calcium, zinc, aluminum, lithium, and nickel. In a particular embodiment, the co-agent is selected from zinc salts of acrylates, diacrylates, methacrylates, and dimethacrylates. In another particular embodiment, the agent is zinc diacrylate (ZDA). When the co-agent is zinc diacrylate and/or zinc dimethacrylate, the co-agent is typically included in the rubber composition in an amount within the range having a lower limit of 1 or 5 or 10 or 15 or 19 or 20 parts by weight per 100 parts of the total rubber, and an upper limit of 24 or 25 or 30 or 35 or 40 or 45 or 50 or 60 parts by weight per 100 parts of the total rubber.

Radical scavengers such as a halogenated organosulfur, organic disulfide, or inorganic disulfide compounds may be added to the polyalkenamer rubber composition to increase the COR at a given compression. Preferred halogenated organosulfur compounds include, but are not limited to, pentachlorothiophenol (PCTP) and salts of PCTP such as zinc pentachlorothiophenol (ZnPCTP). Using PCTP and ZnPCTP in golf ball inner cores helps produce softer and faster inner cores. The PCTP and ZnPCTP compounds help increase the resiliency and the coefficient of restitution of the core. In a particular embodiment, the soft and fast agent is selected from ZnPCTP, PCTP, ditolyl disulfide, diphenyl disulfide, dixylyl disulfide, 2-nitroresorcinol, and combinations thereof.

The polyalkenamer compositions of the present invention also may include "fillers," which are added to adjust the density and/or specific gravity of the material. As used herein, the term "fillers" includes any compound or composition that can be used to adjust the density and/or other properties of the subject golf ball. Suitable fillers include, but are not limited to, polymeric or mineral fillers, metal fillers, metal alloy fillers, metal oxide fillers and carbonaceous fillers. Fillers can be in the form of flakes, fibers, fibrils, or powders. Regrind, which is ground, recycled core material (for example, ground to about 30 mesh particle size), can also be used. The amount and type of fillers utilized are governed by the amount and weight of other ingredients in the golf ball, since a maximum golf ball weight of 45.93 g (1.62 ounces) has been established by the United States Golf Association (USGA). Suitable fillers generally have a specific gravity from about 2 to 20. In one preferred embodiment, the specific gravity can be about 2 to 6.

Suitable polymeric or mineral fillers include, for example, precipitated hydrated silica, clay, talc, asbestos, glass fibers, aramid fibers, mica, calcium metasilicate, barium sulfate, zinc sulfide, lithopone, silicates, silicon carbide, diatomaceous earth, polyvinyl chloride, carbonates such as calcium carbonate and magnesium carbonate. Suitable metal fillers include titanium, tungsten, aluminum, bismuth, nickel, molybdenum, iron, lead, copper, boron, cobalt, beryllium, zinc, and tin. Suitable metal alloys include steel, brass, bronze, boron carbide whiskers, and tungsten carbide whiskers. Suitable metal oxide fillers include zinc oxide, iron oxide, aluminum oxide, titanium oxide, magnesium oxide, and zirconium oxide. Suitable particulate carbonaceous fillers include graphite, carbon black, cotton flock, natural bitumen, cellulose flock, and leather fiber. Micro balloon fillers such as glass and ceramic, and fly ash fillers can also be used.

As discussed above, the rubber compositions may include antioxidants to prevent the breakdown of the elastomers. In addition, the polyalkenamer rubber compositions may optionally include processing aids such as high molecular weight organic acids and salts thereof. Suitable organic acids are aliphatic organic acids, aromatic organic acids, saturated mono-functional organic acids, unsaturated monofunctional organic acids, multi-unsaturated mono-functional organic acids, and dimerized derivatives thereof. Particular examples of suitable organic acids include, but are not limited to, caproic acid, caprylic acid, capric acid, lauric acid, stearic acid, behenic acid, erucic acid, oleic acid, linoleic acid, myristic acid, benzoic acid, palmitic acid, phenylacetic acid, naphthalenoic acid, dimerized derivatives thereof. The organic acids are aliphatic, mono-functional (saturated, unsaturated, or multi-unsaturated) organic acids. Salts of these organic acids may also be employed. The salts of organic acids include the salts of barium, lithium, sodium, zinc, bismuth, chromium, cobalt, copper, potassium, strontium, titanium, tungsten, magnesium, cesium, iron, nickel, silver, aluminum, tin, or calcium, salts of fatty acids, particularly stearic, behenic, erucic, oleic, linoelic or dimerized derivatives thereof. It is preferred that the organic acids and salts of the present invention be relatively non-migratory (they do not bloom to the surface of the polymer under ambient temperatures) and non-volatile (they do not volatilize at temperatures required for melt-blending.)

Other ingredients such as accelerators (for example, tetra methylthiuram), processing aids, dyes and pigments, wetting agents, surfactants, plasticizers, coloring agents, fluorescent agents, chemical blowing and foaming agents, defoaming agents, stabilizers, softening agents, impact modifiers, antioxidants, antiozonants, as well as other additives known in the art may be added to the rubber composition. The core may be formed by mixing and molding the rubber composition using conventional techniques. These cores can be used to make finished golf balls by surrounding the core with outer core layer(s), intermediate layer(s), and/or cover materials as discussed further below.

In one embodiment, the polyalkenamer rubber composition is used to make the inner core layer. In a second embodiment, the polyalkenamer rubber composition is used to make the intermediate core layer; while in a third embodiment, the polyalkenamer rubber composition is used to make the outer core layer. That is, the polyalkenamer rubber composition may be processed as a thermoplastic material and then cross-linked in a post-molding step, or the rubber composition may be processed and cross-linked in an ordinary manner as described above. Alternatively, the polyalkenamer rubber composition may be processed as a thermoplastic material and remain as a thermoplastic material in the final golf ball

construction. In other words, the polyalkenamer rubber composition may be processed as a thermoplastic or thermoset material and used in the center, intermediate, and/or outer core layer. Also, it should be understood the polyalkenamer rubber composition may be used to make more than one core layer. For example, the polyalkenamer rubber composition may be used to make the inner core and outer core layers. In another version, the polyalkenamer rubber composition may be used to make each core layer (inner, intermediate, and outer).

The polyalkenamer rubber materials of this invention may be used with any type of ball construction in accordance with the present invention. Such golf ball designs include, for example, four-piece and five-piece designs. Referring to FIG. 1, one version of a golf ball that can be made in accordance with this invention is generally indicated at (10). The golf ball includes a multi-layered core comprising a center (12), intermediate core layer (14), and outer core layer (16). A cover (18) is disposed about the outer core layer. The golf ball shown in FIG. 1 is for illustrative purposes only and is not meant to be restrictive. It should be recognized that other golf ball constructions can be made in accordance with this invention. For example, in another version, the ball may include a multi-layered cover having inner and outer cover layers. In yet another version, the ball may include an intermediate layer disposed between the core and cover. The intermediate and cover sections may be single or multi-layered.

The core may contain sections having substantially the same hardness or different hardness levels. That is, there can be substantially uniform hardness throughout the different sections or there can be hardness gradients. For example, the inner core layer, intermediate core layer, and outer core layer each may have "positive" hardness gradients (that is, the outer surface of the inner core layer is harder than its geometric center; the outer surface of the intermediate core layer is harder than the inner surface of the intermediate layer; and the outer surface of the outer core layer is harder than the inner surface of the outer core layer.) Other embodiments of golf balls having various combinations of positive, negative, and zero hardness gradients in the inner, intermediate, and outer core layers may be made in accordance with this invention. For example, the inner core may have a positive hardness gradient and the outer core layer may have a negative hardness gradient. In another example, the inner core may have a negative hardness gradient and the outer core layer may have a positive hardness gradient. Other examples include balls wherein the inner core has a positive hardness gradient and the outer core layer has a "zero hardness gradient." (That is, the hardness values of the outer surface of the outer core layer and the inner surface of the outer core layer are substantially the same.) Particularly, the term, "zero hardness gradient" as used herein, means a surface to center Shore C hardness gradient of less than 8, preferably less than 5 and most preferably less than 3 and may be zero or negative 1 to negative 25. The term, "negative hardness gradient" as used herein, means a surface to center Shore C hardness gradient of less than zero. The term, "zero hardness gradient" and the term, "negative hardness gradient" may be used herein interchangeably to refer to hardness gradients of negative 1 to negative 25. The term, "positive hardness gradient" as used herein, means a surface to center Shore C hardness gradient of 8 or greater, preferably 10 or greater, and most preferably 20 or greater.

Golf ball cores of the present invention typically have a coefficient of restitution ("COR") at 125 ft/s of at least 0.750, or at least 0.775 or at least 0.780, or at least 0.782, or at least

19

0.785, or at least 0.787, or at least 0.790, or at least 0.795, or at least 0.798, or at least 0.800.

The multi-layer core is enclosed with a cover, which may be a single-, dual-, or multi-layer cover, preferably having an overall thickness within a range having a lower limit of 0.010 or 0.020 or 0.025 or 0.030 or 0.040 or 0.045 inches and an upper limit of 0.050 or 0.060 or 0.070 or 0.075 or 0.080 or 0.090 or 0.100 or 0.150 or 0.200 or 0.300 or 0.500 inches. In a particular embodiment, the cover is a single layer having a thickness of from 0.025 inches to 0.035 inches. The cover 10 preferably has a surface hardness of 60 Shore D or greater, or 65 Shore D or greater. The cover preferably has a material hardness of 60 Shore D or greater, or 65 Shore D or greater.

Suitable cover materials include, but are not limited to, ionomer resins and blends thereof (e.g., Surlyn® ionomer resins and DuPont® HPF 1000 and HPF 2000, commercially available from E. I. du Pont de Nemours and Company; Iotek® ionomers, commercially available from ExxonMobil Chemical Company; Amplify® JO ionomers of ethylene acrylic acid copolymers, commercially available from The Dow Chemical Company; and Clarix® ionomer resins, commercially available from A. Schulman Inc.); polyurethanes; polyureas; copolymers and hybrids of polyurethane and polyurea; polyethylene, including, for example, low density polyethylene, linear low density polyethylene, and high density polyethylene; polypropylene; rubber-toughened olefin polymers; acid copolymers, e.g., (meth)acrylic acid, which do not become part of an ionomeric copolymer; plastomers; flexomers; styrene/butadiene/styrene block copolymers; styrene/ethylene-butylene/styrene block copolymers; dynamically vulcanized elastomers; ethylene vinyl acetates; ethylene methyl acrylates; polyvinyl chloride resins; polyamides, amide-ester elastomers, and graft copolymers of ionomer and polyamide, including, for example, Pebax® thermoplastic polyether block amides, commercially available from Arkema Inc; crosslinked trans-polyisoprene and blends thereof; polyester-based thermoplastic elastomers, such as Hytrel®, commercially available from E. I. du Pont de Nemours and Company; polyurethane-based thermoplastic elastomers, such as Elastollan®, commercially available from BASF; synthetic or natural vulcanized rubber; and combinations thereof. In a particular embodiment, the cover is a single layer formed from a composition selected from the group consisting of ionomers, polyester elastomers, polyamide elastomers, and combinations of two or more thereof.

Compositions comprising an ionomer or a blend of two or more ionomers are particularly suitable cover materials. Preferred ionomeric cover compositions include:

- (a) a composition comprising a "high acid ionomer" (i.e., having an acid content of greater than 16 wt %), such as Surlyn 8150®;
- (b) a composition comprising a high acid ionomer and a maleic anhydride-grafted non-ionomeric polymer (e.g., Fusabond® functionalized polymers). A particularly preferred blend of high acid ionomer and maleic anhydride-grafted polymer is a 84 wt %/16 wt % blend of Surlyn 8150® and Fusabond®. Blends of high acid ionomers with maleic anhydride-grafted polymers are further disclosed, for example, in U.S. Pat. Nos. 6,992,135 and 6,677,401, the entire disclosures of which are hereby incorporated herein by reference;
- (c) a composition comprising a 50/45/5 blend of Surlyn® 8940/Surlyn® 9650/Nucrel® 960, preferably having a material hardness of from 80 to 85 Shore C;
- (d) a composition comprising a 50/25/25 blend of Surlyn® 8940/Surlyn® 9650/Surlyn® 9910, preferably having a material hardness of about 90 Shore C;

20

(e) a composition comprising a 50/50 blend of Surlyn® 8940/Surlyn® 9650, preferably having a material hardness of about 86 Shore C;

(f) a composition comprising a blend of Surlyn® 7940/Surlyn® 8940, optionally including a melt flow modifier;

(g) a composition comprising a blend of a first high acid ionomer and a second high acid ionomer, wherein the first high acid ionomer is neutralized with a different cation than the second high acid ionomer (e.g., 50/50 blend of Surlyn® 8150 and Surlyn® 9150), optionally including one or more melt flow modifiers such as an ionomer, ethylene-acid copolymer or ester terpolymer; and

(h) a composition comprising a blend of a first high acid ionomer and a second high acid ionomer, wherein the first high acid ionomer is neutralized with a different cation than the second high acid ionomer, and from 0 to 10 wt % of an ethylene/acid/ester ionomer wherein the ethylene/acid/ester ionomer is neutralized with the same cation as either the first high acid ionomer or the second high acid ionomer or a different cation than the first and second high acid ionomers (e.g., a blend of 40-50 wt % Surlyn® 8140, 40-50 wt % Surlyn® 9120, and 0-10 wt % Surlyn® 6320).

Surlyn 8150®, Surlyn® 8940, and Surlyn® 8140 are different grades of E/MAA copolymer in which the acid groups have been partially neutralized with sodium ions. Surlyn® 9650, Surlyn® 9910, Surlyn® 9150, and Surlyn® 9120 are 30 different grades of E/MAA copolymer in which the acid groups have been partially neutralized with zinc ions. Surlyn® 7940 is an E/MAA copolymer in which the acid groups have been partially neutralized with lithium ions. Surlyn® 6320 is a very low modulus magnesium ionomer with a medium acid content. Nucrel® 960 is an E/MAA copolymer resin nominally made with 15 wt % methacrylic acid. Surlyn® ionomers, Fusabond® polymers, and Nucrel® copolymers are commercially available from E. I. du Pont de Nemours and Company.

40 Ionomeric cover compositions can be blended with non-ionic thermoplastic resins, particularly to manipulate product properties. Examples of suitable non-ionic thermoplastic resins include, but are not limited to, polyurethane, poly-ether-ether, poly-amide-ether, polyether-urea, thermoplastic polyether block amides (e.g., Pebax® block copolymers, commercially available from Arkema Inc.), styrene-butadiene-styrene block copolymers, styrene(ethylene-butylene)-styrene block copolymers, polyamides, polyesters, polyolefins (e.g., polyethylene, polypropylene, ethylene-propylene copolymers, polyethylene-(meth)acrylate, polyethylene-(meth)acrylic acid, functionalized polymers with maleic anhydride grafting, Fusabond® functionalized polymers commercially available from E. I. du Pont de Nemours and Company, functionalized polymers with epoxidation, elastomers (e.g., ethylene propylene diene monomer rubber, metallocene-catalyzed polyolefin) and ground powders of thermoset elastomers. Suitable ionomeric cover materials are further disclosed, for example, in U.S. Pat. Nos. 6,653,382, 6,756,436, 6,894,098, 6,919,393, and 6,953,820, the entire disclosures of which are hereby incorporated by reference. Ionomer golf ball cover compositions may include a flow modifier, such as, but not limited to, Nucrel® acid copolymer resins, and particularly Nucrel® 960. Nucrel® acid copolymer resins are commercially available from E. I. du Pont de Nemours and Company.

Polyurethanes, polyureas, and blends, copolymers, and hybrids of polyurethane/polyurea are also particularly suit-

able for forming cover layers. When used as cover layer materials, polyurethanes and polyureas can be thermoset or thermoplastic. Thermoset materials can be formed into golf ball layers by conventional casting or reaction injection molding techniques. Thermoplastic materials can be formed into golf ball layers by conventional compression or injection molding techniques.

Polyurethane cover compositions of the present invention include those formed from the reaction product of at least one polyisocyanate and at least one curing agent. The curing agent can include, for example, one or more diamines, one or more polyols, or a combination thereof. The at least one polyisocyanate can be combined with one or more polyols to form a prepolymer, which is then combined with the at least one curing agent. Thus, when polyols are described herein they may be suitable for use in one or both components of the polyurethane material, i.e., as part of a prepolymer and in the curing agent. The curing agent includes a polyol curing agent preferably selected from the group consisting of ethylene glycol; diethylene glycol; polyethylene glycol; propylene glycol; polypropylene glycol; lower molecular weight polytetramethylene ether glycol; 1,3-bis(2-hydroxyethoxy)benzene; 1,3-bis-[2-(2-hydroxyethoxy)ethoxy]benzene; 1,3-bis-{2-[2-(2-hydroxyethoxy)ethoxy]ethoxy}benzene; 1,4-butanediol; 1,5-pentanediol; 1,6-hexanediol; resorcinol-di-( $\beta$ -hydroxyethyl)ether; hydroquinone-di-( $\beta$ -hydroxyethyl)ether; trimethylol propane; and combinations thereof.

Suitable polyurethane cover compositions of the present invention also include those formed from the reaction product of at least one isocyanate and at least one curing agent or the reaction product of at least one isocyanate, at least one polyol, and at least one curing agent. The polyisocyanate can be combined with one or more polyols to form a prepolymer, which is then combined with the at least one curing agent. Suitable polyurethane cover compositions of the present invention also include those formed from the reaction product of at least one isocyanate and at least one curing agent or the reaction product of at least one isocyanate, at least one polyol, and at least one curing agent. Basically, polyurethane compositions contain urethane linkages formed by reacting an isocyanate group ( $-\text{N}=\text{C}=\text{O}$ ) with a hydroxyl group ( $\text{OH}$ ). Polyurethanes are produced by the reaction of a multi-functional isocyanate with a polyol in the presence of a catalyst and other additives. The chain length of the polyurethane prepolymer is extended by reacting it with a hydroxyl-terminated curing agent. Polyurea compositions, which are distinct from the above-described polyurethanes, also can be formed. In general, polyurea compositions contain urea linkages formed by reacting an isocyanate group ( $-\text{N}=\text{C}=\text{O}$ ) with an amine group ( $\text{NH}$  or  $\text{NH}_2$ ). The chain length of the polyurea prepolymer is extended by reacting the prepolymer with an amine curing agent. Hybrid compositions containing urethane and urea linkages also may be produced. For example, a polyurethane/urea hybrid composition may be produced when a polyurethane prepolymer is reacted with an amine-terminated curing agent. The term, "hybrid polyurethane/polyureas" is also meant to encompass blends and copolymers of polyurethanes and polyureas.

Any method known to one of ordinary skill in the art may be used to combine the polyisocyanate, polyol, and curing agent of the present invention. One commonly employed method, known in the art as a one-shot method, involves concurrent mixing of the polyisocyanate, polyol, and curing agent. This method results in a mixture that is inhomogeneous (more random) and affords the manufacturer less control over the molecular structure of the resultant composition. A preferred method of mixing is known as a prepolymer method. In

this method, the polyisocyanate and the polyol are mixed separately prior to addition of the curing agent. This method affords a more homogeneous mixture resulting in a more consistent polymer composition.

Suitable polyurethanes and polyureas are further disclosed, for example, in U.S. Pat. Nos. 5,334,673; 5,484,870; 6,476,176; 6,506,851; 6,835,794; 6,867,279; 6,958,379; 6,960,630; 6,964,621; 7,041,769; 7,105,623; 7,131,915; and 7,186,777, the entire disclosures of which are hereby incorporated herein by reference. The cover compositions may include a flow modifier, such as, but not limited to, Nucrel® acid copolymer resins, and particularly Nucrel® 960. Nucrel® acid copolymer resins are commercially available from E. I. du Pont de Nemours and Company. The cover compositions may also include one or more filler(s), such as the fillers given above for rubber compositions of the present invention (e.g., titanium dioxide, barium sulfate, etc.), and/or additive(s), such as coloring agents, fluorescent agents, whitening agents, antioxidants, dispersants, UV absorbers, light stabilizers, plasticizers, surfactants, compatibility agents, foaming agents, reinforcing agents, release agents, and the like.

Cover compositions may include one or more filler(s), such as the fillers given above for rubber compositions of the present invention (e.g., titanium dioxide, barium sulfate, etc.), and/or additive(s), such as coloring agents, fluorescent agents, whitening agents, antioxidants, dispersants, UV absorbers, light stabilizers, plasticizers, surfactants, compatibility agents, foaming agents, reinforcing agents, release agents, and the like. Suitable cover materials and constructions also include, but are not limited to, those disclosed in U.S. Pat. Nos. 5,919,100; 6,117,025; 6,767,940; 6,960,630; and 7,182,702, the entire disclosures of which are hereby incorporated herein by reference.

In a particular embodiment, the cover is a single layer, preferably formed from an ionomeric composition, and has a surface hardness of 60 Shore D or greater, a material hardness of 60 Shore D or greater, and a thickness of 0.02 inches or greater or 0.03 inches or greater or 0.04 inches or greater or a thickness within a range having a lower limit of 0.010 or 0.015 or 0.020 inches and an upper limit of 0.035 or 0.040 or 0.050 inches.

In another particular embodiment, the cover is a dual- or multi-layer cover including an inner or intermediate cover layer formed from an ionomeric composition and an outer cover layer formed from a polyurethane- or polyurea-based composition. The ionomeric layer preferably has a surface hardness of 70 Shore D or less, or 65 Shore D or less, or less than 65 Shore D, or a Shore D hardness of from 50 to 65, or a Shore D hardness of from 57 to 60, or a Shore D hardness of 58, and a thickness within a range having a lower limit of 0.010 or 0.020 or 0.030 inches and an upper limit of 0.045 or 0.080 or 0.120 inches. The outer cover layer is preferably formed from a castable or reaction injection moldable polyurethane, polyurea, or copolymer or hybrid of polyurethane/polyurea. Such cover material is preferably thermosetting, but may be thermoplastic. The outer cover layer composition preferably has a material hardness of 85 Shore C or less, or 45 Shore D or less, or 40 Shore D or less, or from 25 Shore D to 40 Shore D, or from 30 Shore D to 40 Shore D. The outer cover layer preferably has a surface hardness within a range having a lower limit of 20 or 30 or 35 or 40 Shore D and an upper limit of 52 or 58 or 60 or 65 or 70 or 72 or 75 Shore D. The outer cover layer preferably has a thickness within a range having a lower limit of 0.010 or 0.015 or 0.025 inches and an upper limit of 0.035 or 0.040 or 0.045 or 0.050 or 0.055 or 0.075 or 0.080 or 0.115 inches. A moisture vapor barrier

layer is optionally employed between the core and the cover. Moisture vapor barrier layers are further disclosed, for example, in U.S. Pat. Nos. 6,632,147, 6,838,028, 6,932,720, 7,004,854, and 7,182,702, the disclosures of which are hereby incorporated by reference.

One or more of the golf ball layers, other than the innermost and outermost layers, is optionally a non-uniform thickness layer. For purposes of the present disclosure, a "non-uniform thickness layer" refers to a layer having projections, webs, ribs, and the like, disposed thereon such that the thickness of the layer varies. The non-uniform thickness layer preferably has one or more of: a plurality of projections disposed thereon, a plurality of a longitudinal webs, a plurality of latitudinal webs, or a plurality of circumferential webs. In a particular embodiment, the non-uniform thickness layer comprises a plurality of projections disposed on the outer surface and/or inner surface thereof. The projections may be made integral with the layer or may be made separately and then attached to the layer. The projections may have any shape or profile including, but not limited to, trapezoidal, sinusoidal, dome, stepped, cylindrical, conical, truncated conical, rectangular, pyramidal with polygonal base, truncated pyramidal or polyhedral. Suitable shapes and profiles for the inner and outer projections also include those disclosed in U.S. Pat. No. 6,293,877, the entire disclosure of which is hereby incorporated herein by reference. In another particular embodiment, the non-uniform thickness layer comprises a plurality of inner and/or outer circular webs disposed thereon. In a particular aspect of this embodiment, the presence of the webs increases the stiffness of the non-uniform thickness layer. The webs may be longitudinal webs, latitudinal webs, or circumferential webs.

Non-uniform thickness layers of golf balls of the present invention preferably have a thickness within a range having a lower limit of 0.010 or 0.015 inches to 0.100 or 0.150 inches, and preferably have a flexural modulus within a range having a lower limit of 5,000 or 10,000 psi and an upper limit of 80,000 or 90,000 psi. Non-uniform thickness layers are further disclosed, for example, in U.S. Pat. No. 6,773,364, the entire disclosure of which is hereby incorporated herein by reference.

In addition to the materials disclosed above, any of the core or cover layers may comprise one or more of the following materials: thermoplastic elastomer, thermoset elastomer, synthetic rubber, thermoplastic vulcanizate, copolymeric ionomer, terpolymeric ionomer, polycarbonate, polyolefin, polyamide, copolymeric polyamide, polyesters, polyester-amides, polyether-amides, polyvinyl alcohols, acrylonitrile-butadiene-styrene copolymers, polyarylate, polyacrylate, polyphenylene ether, impact-modified polyphenylene ether, high impact polystyrene, diallyl phthalate polymer, metallocene-catalyzed polymers, styrene-acrylonitrile (SAN), olefin-modified SAN, acrylonitrile-styrene-acrylonitrile, styrene-maleic anhydride (S/MA) polymer, styrenic copolymer, functionalized styrenic copolymer, functionalized styrenic terpolymer, styrenic terpolymer, cellulose polymer, liquid crystal polymer (LCP), ethylene-propylene-diene rubber (EPDM), ethylene-vinyl acetate copolymer (EVA), ethylene propylene rubber (EPR), ethylene vinyl acetate, polyurea, and polysiloxane. Suitable polyamides for use as an additional material in compositions disclosed herein also include resins obtained by: (1) polycondensation of (a) a dicarboxylic acid, such as oxalic acid, adipic acid, sebacic acid, terephthalic acid, isophthalic acid or 1,4-cyclohexanedicarboxylic acid, with (b) a diamine, such as ethylenediamine, tetramethylenediamine, pentamethylenediamine, hexamethylenediamine, or decamethylenediamine, 1,4-cyclohexyldiamine or

m-xylylenediamine; (2) a ring-opening polymerization of cyclic lactam, such as  $\epsilon$ -caprolactam or  $\omega$ -laurolactam; (3) polycondensation of an aminocarboxylic acid, such as 6-aminocaproic acid, 9-aminononanoic acid, 11-aminoundecanoic acid or 12-aminododecanoic acid; or (4) copolymerization of a cyclic lactam with a dicarboxylic acid and a diamine. Specific examples of suitable polyamides include Nylon 6, Nylon 66, Nylon 610, Nylon 11, Nylon 12, copolymerized Nylon, Nylon MXD6, and Nylon 46.

Other preferred materials suitable for use as an additional material in golf ball compositions disclosed herein include Skypel polyester elastomers, commercially available from SK Chemicals of South Korea; Septon® diblock and triblock copolymers, commercially available from Kuraray Corporation of Kurashiki, Japan; and Kraton® diblock and triblock copolymers, commercially available from Kraton Polymers LLC of Houston, Tex.

Ionomers are also well suited for blending with compositions disclosed herein. Suitable ionomeric polymers include  $\alpha$ -olefin/unsaturated carboxylic acid copolymer- or terpolymer-type ionomeric resins. Copolymeric ionomers are obtained by neutralizing at least a portion of the carboxylic groups in a copolymer of an  $\alpha$ -olefin and an  $\alpha,\beta$ -unsaturated carboxylic acid having from 3 to 8 carbon atoms, with a metal ion. Terpolymeric ionomers are obtained by neutralizing at least a portion of the carboxylic groups in a terpolymer of an  $\alpha$ -olefin, an  $\alpha,\beta$ -unsaturated carboxylic acid having from 3 to 8 carbon atoms, and an  $\alpha,\beta$ -unsaturated carboxylate having from 2 to 22 carbon atoms, with a metal ion. Examples of suitable  $\alpha$ -olefins for copolymeric and terpolymeric ionomers include ethylene, propylene, 1-butene, and 1-hexene. Examples of suitable unsaturated carboxylic acids for copolymeric and terpolymeric ionomers include acrylic, methacrylic, ethacrylic,  $\alpha$ -chloroacrylic, crotonic, maleic, fumaric, and itaconic acid. Copolymeric and terpolymeric ionomers include ionomers having varied acid contents and degrees of acid neutralization, neutralized by monovalent or bivalent cations as disclosed herein. Examples of commercially available ionomers suitable for blending with compositions disclosed herein include Surlyn® ionomer resins, commercially available from E. I. du Pont de Nemours and Company, and Iotek® ionomers, commercially available from ExxonMobil Chemical Company.

Silicone materials are also well suited for blending with compositions disclosed herein. Suitable silicone materials include monomers, oligomers, prepolymers, and polymers, with or without adding reinforcing filler. One type of silicone material that is suitable can incorporate at least 1 alkenyl group having at least 2 carbon atoms in their molecules. Examples of these alkenyl groups include, but are not limited to, vinyl, allyl, butenyl, pentenyl, hexenyl, and decenyl. The alkenyl functionality can be located at any location of the silicone structure, including one or both terminals of the structure. The remaining (i.e., non-alkenyl) silicon-bonded organic groups in this component are independently selected from hydrocarbon or halogenated hydrocarbon groups that contain no aliphatic unsaturation. Non-limiting examples of these include: alkyl groups, such as methyl, ethyl, propyl, butyl, pentyl, and hexyl; cycloalkyl groups, such as cyclohexyl and cycloheptyl; aryl groups, such as phenyl, tolyl, and xylyl; aralkyl groups, such as benzyl and phenethyl; and halogenated alkyl groups, such as 3,3,3-trifluoropropyl and chloromethyl. Another type of suitable silicone material is one having hydrocarbon groups that lack aliphatic unsaturation. Specific examples include: trimethylsiloxy-blocked dimethylsiloxane-methylhexenylsiloxane copolymers; dimethylhexenylsiloxy-blocked dimethylsiloxane-methyl-

hexenylsiloxane copolymers; trimethylsiloxy-endblocked dimethylsiloxane-methylvinylsiloxane copolymers; trimethylsiloxy-endblocked methylphenylsiloxane-dimethylsiloxane-methylvinylsiloxane copolymers; dimethylvinylsiloxo-endblocked dimethylpolysiloxanes; dimethylvinylsiloxo-endblocked dimethylsiloxane-methylvinylsiloxane copolymers; dimethylvinylsiloxo-endblocked methylphenylpolysiloxanes; dimethylvinylsiloxo-endblocked methylphenylsiloxane-dimethylsiloxane-methylvinylsiloxane copolymers; and the copolymers listed above wherein at least one group is dimethylhydroxysiloxyl. Examples of commercially available silicones suitable for blending with compositions disclosed herein include Silastic® silicone rubber, commercially available from Dow Corning Corporation of Midland, Mich.; Blensil® silicone rubber, commercially available from General Electric Company of Waterford, N.Y.; and Elastosil® silicones, commercially available from Wacker Chemie AG of Germany.

Other types of copolymers can also be added to the golf ball compositions disclosed herein. For example, suitable copolymers comprising epoxy monomers include styrene-butadiene-styrene block copolymers in which the polybutadiene block contains an epoxy group, and styrene-isoprene-styrene block copolymers in which the polyisoprene block contains epoxy. Examples of commercially available epoxy functionalized copolymers include ESBS A1005, ESBS A1010, ESBS A1020, ESBS AT018, and ESBS AT019 epoxidized styrene-butadiene-styrene block copolymers, commercially available from Daicel Chemical Industries, Ltd. Of Japan.

Ionomeric compositions used to form golf ball layers of the present invention can be blended with non-ionic thermoplastic resins, particularly to manipulate product properties. Examples of suitable non-ionic thermoplastic resins include, but are not limited to, polyurethane, poly-ether-ester, polyamide-ether, polyether-urea, Pebax® thermoplastic polyether block amides commercially available from Arkema Inc., styrene-butadiene-styrene block copolymers, styrene (ethylene-butylene)-styrene block copolymers, polyamides, polyesters, polyolefins (e.g., polyethylene, polypropylene, ethylene-propylene copolymers, ethylene-(meth)acrylate, ethylene-(meth)acrylic acid, functionalized polymers with maleic anhydride grafting, epoxidation, etc., elastomers (e.g., EPDM, metallocene-catalyzed polyethylene) and ground powders of the thermoset elastomers. Compositions disclosed herein can be either foamed or filled with density adjusting materials to provide desirable golf ball performance characteristics.

The present invention is not limited by any particular process for forming the golf ball layer(s). It should be understood that the layer(s) can be formed by any suitable technique, including injection molding, compression molding, casting, and reaction injection molding. In particular, the relatively thin outer core layer may be formed by any conventional means for forming a thin thermosetting layer comprising a vulcanized or otherwise crosslinked diene rubber including, but not limited to, compression molding, rubber-injection molding, casting of a liquid rubber, and laminating.

When injection molding is used, the composition is typically in a pelletized or granulated form that can be easily fed into the throat of an injection molding machine wherein it is melted and conveyed via a screw in a heated barrel at temperatures of from 150° F. to 600° F., preferably from 200° F. to 500° F. The molten composition is ultimately injected into a closed mold cavity, which may be cooled, at ambient or at an elevated temperature, but typically the mold is cooled to a temperature of from 50° F. to 70° F. After residing in the closed mold for a time of from 1 second to 300 seconds,

preferably from 20 seconds to 120 seconds, the core and/or core plus one or more additional core or cover layers is removed from the mold and either allowed to cool at ambient or reduced temperatures or is placed in a cooling fluid such as water, ice water, dry ice in a solvent, or the like.

When compression molding is used to form a core, the composition is first formed into a preform or slug of material, typically in a cylindrical or roughly spherical shape at a weight slightly greater than the desired weight of the molded core. Prior to this step, the composition may be first extruded or otherwise melted and forced through a die after which it is cut into a cylindrical preform. The preform is then placed into a compression mold cavity and compressed at a mold temperature of from 150° F. to 400° F., preferably from 250° F. to 400° F., and more preferably from 300° F. to 400° F. When compression molding a cover layer, half-shells of the cover layer material are first formed via injection molding. A core is then enclosed within two half-shells, which is then placed into a compression mold cavity and compressed. Reaction injection molding processes are further disclosed, for example, in U.S. Pat. Nos. 6,083,119, 7,208,562, 7,281,997, 7,282,169, 7,338,391, the entire disclosures of which are hereby incorporated herein by reference. Thermoplastic layers herein may be treated in such a manner as to create a positive or negative hardness gradient. In golf ball layers of the present invention wherein a thermosetting rubber is used, gradient-producing processes and/or gradient-producing rubber formulation may be employed.

Golf balls of the present invention typically have a coefficient of restitution (COR) of 0.700 or greater, preferably 0.750 or greater, and more preferably 0.780 or greater. Golf balls of the present invention typically have a compression of 40 or greater, or a compression within a range having a lower limit of 50 or 60 and an upper limit of 100 or 120. Golf balls of the present invention will typically have dimple coverage of 60% or greater, preferably 65% or greater, and more preferably 75% or greater. The test methods for measuring COR and compression are described in further detail below. The United States Golf Association specifications limit the minimum size of a competition golf ball to 1.680 inches. There is no specification as to the maximum diameter, and golf balls of any size can be used for recreational play. Golf balls of the present invention can have an overall diameter of any size. The preferred diameter of the present golf balls is within a range having a lower limit of 1.680 inches and an upper limit of 1.740 or 1.760 or 1.780 or 1.800 inches.

Golf balls of the present invention preferably have a moment of inertia ("MOI") of 70-95 g·cm<sup>2</sup>, preferably 75-93 g·cm<sup>2</sup>, and more preferably 76-90 g·cm<sup>2</sup>. For low MOI embodiments, the golf ball preferably has an MOI of 85 g·cm<sup>2</sup> or less, or 83 g·cm<sup>2</sup> or less. For high MOI embodiments, the golf ball preferably has an MOI of 86 g·cm<sup>2</sup> or greater, or 87 g·cm<sup>2</sup> or greater. Methods for measuring MOI are described in further detail below.

#### 55 Test Methods

**Hardness.** The center hardness of a core is obtained according to the following procedure. The core is gently pressed into a hemispherical holder having an internal diameter approximately slightly smaller than the diameter of the core, such that the core is held in place in the hemispherical portion of the holder while concurrently leaving the geometric central plane of the core exposed. The core is secured in the holder by friction, such that it will not move during the cutting and grinding steps, but the friction is not so excessive that distortion of the natural shape of the core would result. The core is secured such that the parting line of the core is roughly parallel to the top of the holder. The diameter of the core is

measured 90 degrees to this orientation prior to securing. A measurement is also made from the bottom of the holder to the top of the core to provide a reference point for future calculations. A rough cut is made slightly above the exposed geometric center of the core using a band saw or other appropriate cutting tool, making sure that the core does not move in the holder during this step. The remainder of the core, still in the holder, is secured to the base plate of a surface grinding machine. The exposed 'rough' surface is ground to a smooth, flat surface, revealing the geometric center of the core, which can be verified by measuring the height from the bottom of the holder to the exposed surface of the core, making sure that exactly half of the original height of the core, as measured above, has been removed to within  $\pm 0.004$  inches. Leaving the core in the holder, the center of the core is found with a center square and carefully marked and the hardness is measured at the center mark according to ASTM D-2240. Additional hardness measurements at any distance from the center of the core can then be made by drawing a line radially outward from the center mark, and measuring the hardness at any given distance along the line, typically in 2 mm increments from the center. The hardness at a particular distance from the center should be measured along at least two, preferably four, radial arms located 180° apart, or 90° apart, respectively, and then averaged. All hardness measurements performed on a plane passing through the geometric center are performed while the core is still in the holder and without having disturbed its orientation, such that the test surface is constantly parallel to the bottom of the holder, and thus also parallel to the properly aligned foot of the durometer.

The outer surface hardness of a golf ball layer is obtained from the average of a number of measurements taken from opposing hemispheres, taking care to avoid making measurements on the parting line of the core or on surface defects, such as holes or protrusions. Hardness measurements are made pursuant to ASTM D-2240 "Indentation Hardness of Rubber and Plastic by Means of a Durometer." Because of the curved surface, care must be taken to insure that the golf ball or golf ball subassembly is centered under the durometer indenter before a surface hardness reading is obtained. A calibrated, digital durometer, capable of reading to 0.1 hardness units is used for the hardness measurements. The digital durometer must be attached to, and its foot made parallel to, the base of an automatic stand. The weight on the durometer and attack rate conform to ASTM D-2240. Hardness points should only be measured once at any particular geometric location.

In certain embodiments, a point or plurality of points measured along the "positive" or "negative" gradients may be above or below a line fit through the gradient and its outermost and innermost hardness values. In an alternative preferred embodiment, the hardest point along a particular steep "positive" or "negative" gradient may be higher than the value at the innermost portion of the inner core (the geometric center) or outer core layer (the inner surface)—as long as the outermost point (i.e., the outer surface of the inner core) is greater than (for "positive") or lower than (for "negative") the innermost point (i.e., the geometric center of the inner core or the inner surface of the outer core layer), such that the "positive" and "negative" gradients remain intact.

As discussed above, the direction of the hardness gradient of a golf ball layer is defined by the difference in hardness measurements taken at the outer and inner surfaces of a particular layer. The center hardness of an inner core and hardness of the outer surface of an inner core in a single-core ball or outer core layer are readily determined according to the test procedures provided above. The outer surface of the inner

core layer (or other optional intermediate core layers) in a dual-core ball are also readily determined according to the procedures given herein for measuring the outer surface hardness of a golf ball layer, if the measurement is made prior to surrounding the layer with an additional core layer. Once an additional core layer surrounds a layer of interest, the hardness of the inner and outer surfaces of any inner or intermediate layers can be difficult to determine. Therefore, for purposes of the present invention, when the hardness of the inner or outer surface of a core layer is needed after the inner layer has been surrounded with another core layer, the test procedure described above for measuring a point located 1 mm from an interface is used.

Also, it should be understood that there is a fundamental difference between "material hardness" and "hardness as measured directly on a golf ball." For purposes of the present invention, material hardness is measured according to ASTM D2240 and generally involves measuring the hardness of a flat "slab" or "button" formed of the material. Surface hardness as measured directly on a golf ball (or other spherical surface) typically results in a different hardness value. The difference in "surface hardness" and "material hardness" values is due to several factors including, but not limited to, ball construction (that is, core type, number of cores and/or cover layers, and the like); ball (or sphere) diameter; and the material composition of adjacent layers. It also should be understood that the two measurement techniques are not linearly related and, therefore, one hardness value cannot easily be correlated to the other. Shore C hardness is measured according to the test methods D-2240 as described above.

Moment of Inertia Golf balls of the present invention preferably have a Moment of Inertia ("MOI") of 70-95 g·cm<sup>2</sup>, preferably 75-93 g·cm<sup>2</sup>, and more preferably 76-90 g·cm<sup>2</sup>. For low MOI embodiments, the golf ball preferably has an MOI of 85 g·cm<sup>2</sup> or less, or 83 g·cm<sup>2</sup> or less. For high MOI embodiments, the golf ball preferably has an MOI of 86 g·cm<sup>2</sup> or greater, or 87 g·cm<sup>2</sup> or greater. MOI is measured on a model MOI-005-104 Moment of Inertia Instrument manufactured by Inertia Dynamics of Collinsville, Conn. The instrument is connected to a PC for communication via a COMM port and is driven by MOI Instrument Software Version #1.2.

Compression. As disclosed in Jeff Dalton's Compression by Any Other Name, Science and Golf IV, Proceedings of the World Scientific Congress of Golf (Eric Thain ed., Routledge, 2002) ("J. Dalton"), several different methods can be used to measure compression, including Atti compression, Riehle compression, load/deflection measurements at a variety of fixed loads and offsets, and effective modulus. For purposes of the present invention, "compression" refers to Atti compression and is measured according to a known procedure, using an Atti compression test device, wherein a piston is used to compress a ball against a spring. The travel of the piston is fixed and the deflection of the spring is measured. The measurement of the deflection of the spring does not begin with its contact with the ball; rather, there is an offset of approximately the first 1.25 mm (0.05 inches) of the spring's deflection. Very low stiffness cores will not cause the spring to deflect by more than 1.25 mm and therefore have a zero compression measurement. The Atti compression tester is designed to measure objects having a diameter of 42.7 mm (1.68 inches); thus, smaller objects, such as golf ball cores, must be shimmed to a total height of 42.7 mm to obtain an accurate reading. Conversion from Atti compression to Riehle (cores), Riehle (balls), 100 kg deflection, 130-10 kg deflection or effective modulus can be carried out according to the formulas given in J. Dalton.

Coefficient of Restitution ("COR"). The COR is determined according to a known procedure, wherein a golf ball or golf ball subassembly (for example, a golf ball core) is fired from an air cannon at two given velocities and a velocity of 125 ft/s is used for the calculations. Ballistic light screens are located between the air cannon and steel plate at a fixed distance to measure ball velocity. As the ball travels toward the steel plate, it activates each light screen and the ball's time period at each light screen is measured. This provides an incoming transit time period which is inversely proportional to the ball's incoming velocity. The ball makes impact with the steel plate and rebounds so it passes again through the light screens. As the rebounding ball activates each light screen, the ball's time period at each screen is measured. This provides an outgoing transit time period which is inversely proportional to the ball's outgoing velocity. The COR is then calculated as the ratio of the ball's outgoing transit time period to the ball's incoming transit time period (COR=V<sub>out</sub>N<sub>in</sub>=T<sub>in</sub>/T<sub>out</sub>).

### EXAMPLES

The invention is further illustrated by the following examples, but these examples should not be construed as limiting the scope of the invention.

#### Example 1

In this Example, a slug of a rubber composition having the formulation described in Table 1 was cured at about 330° F. for about 11 minutes to make a solid, single-layered core. The resulting core had a center hardness of about 68 Shore C and a surface hardness of about 70 Shore C. In addition, the core had a compression of about 70 and a COR of about 0.775@125 f/s (1.550 inch diameter solid sphere). When the core was cured at about 350° F. for about 11 minutes, the compression increased to about 90 and the COR increased to about 0.790@125 f/s (1.550 inch diameter solid sphere).

TABLE 1

| Core Composition                                                             | Concentration (parts per hundred) |
|------------------------------------------------------------------------------|-----------------------------------|
| Vestenamer ® 8012 - polyoctenamer rubber available from Evonik Degussa GmbH. | 100                               |
| Zinc diacrylate (ZDA) co-agent                                               | 50                                |
| Zinc oxide (ZnO) filler                                                      | 6                                 |
| Trigonox 145 free-radical initiator                                          | 1.5                               |
| * peroxide free-radical initiator available from Akzo Nobel.                 |                                   |
| Zinc pentachlorothiophenol (ZnPCTP)                                          | 1                                 |

#### Example 2

In this Example, slugs of different polyalkenamer rubber compositions having the formulations described in Table 2 were cured at different temperature/time cycles as described in Table 3 to make solid, single-layered core samples. Concentrations are in parts per hundred (phr) unless otherwise indicated. As used herein, the term "parts per hundred," also known as "phr," is defined as the number of parts by weight of a particular component present in a mixture, relative to 100 parts by weight of the base rubber component. Mathematically, this can be expressed as the weight of an ingredient divided by the total weight of the polymer, multiplied by a factor of 100.

TABLE 2

| (Core Compositions Containing 100% Polyalkenamer as Base Rubber) |                         |                    |                                       |                         |                           |
|------------------------------------------------------------------|-------------------------|--------------------|---------------------------------------|-------------------------|---------------------------|
| Sample                                                           | Base Rubber             | ZDA Co-agent (phr) | Peroxide Free-Radical Initiator (phr) | Zinc Oxide Filler (phr) | Soft and Fast Agent (phr) |
| A                                                                | Vestenamer* 8012        | 0                  | 0                                     | 0                       | 0                         |
| B                                                                | Vestenamer 8012         | 0                  | 2.50 parts Varox* 231-XL              | 0                       | 0                         |
| C                                                                | Vestenamer 8012         | 0                  | 5.00 parts Varox 231-XL               | 0                       | 0                         |
| D                                                                | Vestenamer 8012 SR-526* | 33.5 parts         | 0.85 parts Perkadox* BC               | 19.9 parts ZnO*         | 0                         |
| E                                                                | Vestenamer 8012 SR-526  | 33.5 parts         | 1.75 parts Perkadox BC                | 19.9 parts ZnO          | 0                         |
| F                                                                | Vestenamer 8012 SR-526  | 33.5 parts         | 3.00 parts Perkadox BC                | 19.9 parts ZnO          | 0                         |
| G                                                                | Vestenamer 8012 SR-526  | 33.5 parts         | 5.00 parts Perkadox BC                | 19.9 parts ZnO          | 0                         |
| H                                                                | Vestenamer 8012 SR-526  | 33.5 parts         | 5.00 parts Perkadox BC                | 19.9 parts ZnO          | 1.0 parts ZnPCTP*         |
| I                                                                | Vestenamer 8012 SR-526  | 50 parts           | 1.00 parts Perkadox BC                | 13.0 parts ZnO          | 1.0 parts ZnPCTP          |
| J                                                                | Vestenamer 8012 SR-526  | 50 parts           | 1.00 parts Perkadox BC                | 13.0 parts ZnO          | 1.0 parts ZnPCTP          |
| K                                                                | Vestenamer 8012 SR-526  | 50 parts           | 2.00 parts Perkadox BC                | 13.0 parts ZnO          | 1.0 parts ZnPCTP          |
| L                                                                | Vestenamer 8012 SR-526  | 50 parts           | 2.00 parts Perkadox BC                | 13.0 parts ZnO          | 1.0 parts ZnPCTP          |

\*Vestenamer ®-8012 polyoctenamer rubber having a trans-content of approximately 80% and a melting point of approximately 54° C., available from Evonik Degussa GmbH.

\*SR-526-zinc diacrylate available from Akzo Nobel NV.

\*Varox ® 231-XL-1,1-di(t-butylperoxy)-3,5-trimethylcyclohexane available from Atofina.

\*Perkadox ® BC-dicumyl peroxide granules available from Akzo Nobel NV.

\*ZnO-zinc oxide

\*ZnPCTP-zinc pentachlorothiophenol, available from Strukol Company and Echina.

TABLE 3

| (Curing Cycle and Properties for Core Samples) |                  |                     |                   |       |                  |
|------------------------------------------------|------------------|---------------------|-------------------|-------|------------------|
| Sample                                         | Cure Temp (° F.) | Cure Time (Minutes) | DCM (Compression) | COR   | Shore C Hardness |
| A                                              | No Heat-Curing   | No Heat-Curing      | 102               | 0.568 | 75               |
| B                                              | 350° F.          | 12 Min.             | 47                | 0.617 | 41               |
| C                                              | 350° F.          | 12 Min.             | -62               | 0.687 | —                |
| D                                              | 350° F.          | 11 Min.             | 60                | 0.767 | 80.4             |
| E                                              | 350° F.          | 11 Min.             | 68                | 0.778 | 82.9             |
| F                                              | 350° F.          | 11 Min.             | 79                | —     | 85.9             |
| G                                              | 350° F.          | 11 Min.             | 75                | 0.780 | 87.6             |
| H                                              | 350° F.          | 11 Min.             | 56                | 0.788 | 83.8             |
| I                                              | 330° F.          | 11 Min.             | 91                | 0.794 | 85.9             |
| J                                              | 350° F.          | 11 Min.             | 94                | 0.795 | 89               |
| K                                              | 330° F.          | 11 Min.             | 98                | 0.792 | 90.7             |
| L                                              | 350° F.          | 11 Min.             | 99                | 0.796 | 90.7             |

#### Example 3

In this Example, slugs of different polyalkenamer rubber compositions having the formulations described in Table 4 were cured at different temperature/time cycles as described in Table 5 to make solid, single-layered core samples.

TABLE 4

| (Core Compositions Containing Blends of Polyalkenamer and Polybutadiene Rubber) |                                |                           |                    |                                       |                         |                           |
|---------------------------------------------------------------------------------|--------------------------------|---------------------------|--------------------|---------------------------------------|-------------------------|---------------------------|
| Sample                                                                          | Base Rubber                    | Secondary Rubber          | ZDA Co-agent (phr) | Peroxide Free-Radical Initiator (phr) | Zinc Oxide Filler (phr) | Soft and Fast Agent (phr) |
| M                                                                               | 80 parts<br>Vestenamer<br>8012 | 20 parts<br>Buna CB<br>23 | 40 parts<br>SR-526 | 1 part<br>Perkadox<br>BC              | 23.5 parts<br>ZnO       | 1 part<br>ZnPCTP          |
| N                                                                               | 80 parts<br>Vestenamer<br>8012 | 20 parts<br>Buna CB<br>23 | 40 parts<br>SR-526 | 1 part<br>Perkadox<br>BC              | 23.5 parts<br>ZnO       | 1 part<br>ZnPCTP          |
| O                                                                               | 80 parts<br>Vestenamer<br>8012 | 20 parts<br>Buna CB<br>23 | 40 parts<br>SR-526 | 3 parts<br>Perkadox<br>BC             | 23.5 parts<br>ZnO       | 1 part<br>ZnPCTP          |
| P                                                                               | 80 parts<br>Vestenamer<br>8012 | 20 parts<br>Buna CB<br>23 | 40 parts<br>SR-526 | 3 parts<br>Perkadox<br>BC             | 23.5 parts<br>ZnO       | 1 part<br>ZnPCTP          |
| Q                                                                               | 80 parts<br>Vestenamer<br>8012 | 20 parts<br>Buna CB<br>23 | 30 parts<br>SR-526 | 1 part<br>Perkadox<br>BC              | 26 parts<br>ZnO         | 2 parts<br>ZnPCTP         |
| R                                                                               | 80 parts<br>Vestenamer<br>8012 | 20 parts<br>Buna CB<br>23 | 30 parts<br>SR-526 | 1 part<br>Perkadox<br>BC              | 26 parts<br>ZnO         | 2 parts<br>ZnPCTP         |
| S                                                                               | 80 parts<br>Vestenamer<br>8012 | 20 parts<br>Buna CB<br>23 | 30 parts<br>SR-526 | 2 parts<br>Perkadox<br>BC             | 26 parts<br>ZnO         | 2 parts<br>ZnPCTP         |
| T                                                                               | 80 parts<br>Vestenamer<br>8012 | 20 parts<br>Buna CB<br>23 | 30 parts<br>SR-526 | 2 parts<br>Perkadox<br>BC             | 26 parts<br>ZnO         | 2 parts<br>ZnPCTP         |

\* Buna ® CB-23 - polybutadiene rubber available from Lanxess Corp.

TABLE 5

| (Curing Cycle and Properties for Core Samples) |                  |                     |                   |       |                  |
|------------------------------------------------|------------------|---------------------|-------------------|-------|------------------|
| Sample                                         | Cure Temp (° F.) | Cure Time (Minutes) | DCM (Compression) | COR   | Shore C Hardness |
| M                                              | 350° F.          | 11 Min.             | 89                | 0.789 | 51.4             |
| N                                              | 330° F.          | 11 Min.             | 89                | 0.788 | 51.7             |
| O                                              | 350° F.          | 11 Min.             | 99                |       | 58.9             |
| P                                              | 330° F.          | 11 Min.             | 96                |       | 58.6             |
| Q                                              | 350° F.          | 11 Min.             | 51                | 0.778 | 43.2             |
| R                                              | 330° F.          | 15 Min.             | 54                | 0.780 | 44.5             |
| S                                              | 350° F.          | 11 Min.             | 57                | 0.780 | 46.9             |
| T                                              | 330° F.          | 15 Min.             | 59                | 0.780 | 48.6             |

In above Tables 2 and 3, the sample cores are made of rubber compositions containing 100% Vestenamer® 8012—polyoctenamer rubber (Samples A-L), while in Tables 4 and 5, the sample cores (M-T) are made of rubber compositions containing 80% Vestenamer 8012 and 20% Buna CB 23-polybutadiene rubber (Samples M-T).

In each of the samples, when the peroxide free-radical initiator is added to the rubber composition and heat and pressure are applied, a complex curing reaction occurs. In general, the resulting cross-linked core compositions have higher COR values. Cores with higher COR values have higher rebound velocities. These high COR cores (and golf balls made with such cores) generally rebound faster, retain more total energy when struck with a club, and have longer flight distance. The relatively high resiliency of the core means that it will reach a higher velocity when struck by a golf club and travel longer distances.

Surprisingly, however, the compression of the polyalkenamer rubber core composition in the above inventive samples does not increase substantially as the COR increases, as would be expected with conventional polybutadiene rubber cores. Rather, the compression of the polyalkenamer rubber

core remains substantially the same or is reduced as the COR increases. While not wishing to be bound by any theory, it is believed the high crystallinity of the polyalkenamer rubber is reduced by adding the peroxide, particularly at relatively high amounts, as shown in Samples C and H (5 phr peroxide), and curing the composition so the rubber chains are cross-linked. This may cause the compression or stiffness of the polyalkenamer rubber composition to be reduced. Adding the peroxide

at these high levels and curing and cross-linking the composition may disrupt the crystallinity of polyalkenamer. The material becomes softer and more rubbery, and the compression of the core sample is reduced. The compression of the core affects the “feel” of the ball as the club face makes

impact with the ball. In general, cores with relatively low compression values have a softer feel. Golf balls made with such cores tend to have better playability and the sensation of hitting such balls is generally more pleasant. Furthermore, in general, when the ball contains a relatively soft core, the resulting spin rate of the ball is relatively low. The compressive force acting on the ball is less when the cover is compressed by the club face against a relatively soft core.

Other than in the operating examples, or unless otherwise expressly specified, all of the numerical ranges, amounts, values and percentages such as those for amounts of materials and others in the specification may be read as if prefaced by the word “about” even though the term “about” may not expressly appear with the value, amount or range. Accordingly, unless indicated to the contrary, the numerical parameters set forth in the specification and attached claims are approximations that may vary depending upon the desired properties sought to be obtained by the present invention. At the very least, and not as an attempt to limit the application of the doctrine of equivalents to the scope of the claims, each numerical parameter should at least be construed in light of the number of reported significant digits and by applying ordinary rounding techniques.

Notwithstanding that the numerical ranges and parameters setting forth the broad scope of the invention are approximations, the numerical values set forth in the specific examples are reported as precisely as possible. Any numerical value, however, inherently contain certain errors necessarily resulting from the standard deviation found in their respective testing measurements. Furthermore, when numerical ranges of varying scope are set forth herein, it is contemplated that any combination of these values inclusive of the recited values may be used.

While it is apparent that the illustrative embodiments of the invention disclosed herein fulfill the objective stated above, it is appreciated that numerous modifications and other embodiments may be devised by those skilled in the art. Therefore, it will be understood that the appended claims are intended to cover all such modifications and embodiments, which would come within the spirit and scope of the present invention.

We claim:

1. A golf ball comprising:
  - an inner core layer having an outer surface and geometric center, the inner core being formed from a first thermoset rubber composition and having a diameter of from 1.000 inches to 1.580 inches, wherein the outer surface hardness is 50 Shore C to 85 Shore C and the center hardness is 40 Shore C to 65 Shore C;
  - an intermediate core layer formed from a thermoplastic composition and having a thickness of 0.005 inches to 0.100 inches and a surface hardness of 50 Shore D to 90 Shore D;
  - an outer core layer formed from a second thermoset rubber composition and having a thickness of 0.010 inches to 0.100 inches and an outer surface hardness that is greater than the Shore C outer surface hardness of the inner core layer; and
  - a cover layer having a thickness of from 0.010 inches to 0.050 inches and a surface hardness of 60 Shore C or greater;
- wherein at least one of the center, intermediate core layer, and outer core layer comprises a polyalkenamer rubber composition, the polyalkenamer being present in the composition in an amount of at least 50 weight percent.
2. The golf ball of claim 1, wherein the specific gravity of at least one of the center, intermediate core layer, and outer core layer is less than 1.05 g/cc.
3. The golf ball of claim 1, wherein the center has a specific gravity of greater than 1.25 g/cc.
4. The golf ball of claim 1, wherein the compression of the inner core layer is 80 or less.
5. The golf ball of claim 4, wherein the compression of the inner core layer is 50 or less.
6. The golf ball of claim 1, wherein the intermediate core layer has a surface hardness of 60 Shore D or less.
7. The golf ball of claim 1, wherein the intermediate core layer has a surface hardness of 60 Shore D or greater.
8. The golf ball of claim 1, wherein the outer core layer has a thickness of 0.035 inches to 0.075 inches.
9. The golf ball of claim 1, wherein the outer core layer has an outer surface hardness of 70 Shore C or greater.
10. The golf ball of claim 9, wherein the outer core layer has an outer surface hardness of 90 Shore C or greater.
11. The golf ball of claim 1, wherein the cover layer comprises an inner cover layer and an outer cover layer.
12. The golf ball of claim 11, wherein the inner cover layer has a material hardness greater than the material hardness of the outer cover layer.
13. A golf ball comprising:
  - an inner core layer having an outer surface and geometric center, the inner core being formed from a first thermoset rubber composition and having a diameter of from 1.000 inches to 1.580 inches, wherein the outer surface hardness is 50 Shore C to 95 Shore C and the center hardness is 40 Shore C to 75 Shore C;
  - an intermediate core layer formed from a thermoplastic composition and having a thickness of 0.005 inches to 0.100 inches and a surface hardness of 50 Shore D to 90 Shore D;
  - an outer core layer formed from a second thermoset rubber composition and having a thickness of 0.010 inches to 0.100 inches and an outer surface hardness that is less than the Shore C outer surface hardness of the inner core layer; and
  - a cover layer having a thickness of from 0.010 inches to 0.050 inches and a surface hardness of 60 Shore C or greater;
- wherein at least one of the center, intermediate core layer, and outer core layer comprises a polyalkenamer rubber composition, the polyalkenamer being present in the composition in an amount of at least 50 weight percent.
14. The golf ball of claim 13, wherein the specific gravity of at least one of the center, intermediate core layer, and outer core layer is less than 1.05 g/cc.
15. The golf ball of claim 13, wherein the center has a specific gravity of greater than 1.25 g/cc.
16. The golf ball of claim 13, wherein the outer core layer has an outer surface hardness of 90 Shore C or less.
17. The golf ball of claim 13, wherein the outer core layer has an outer surface hardness of 85 Shore C or less.
18. The golf ball of claim 13, wherein the outer core layer has a thickness of 0.035 inches to 0.075 inches.
19. The golf ball of claim 13, wherein the cover layer comprises an inner cover layer and an outer cover layer.
20. The golf ball of claim 13, wherein the inner cover layer has a material hardness greater than the material hardness of the outer cover layer.

\* \* \* \* \*